



US008105447B2

(12) **United States Patent**  
**Oikawa et al.**

(10) **Patent No.:** **US 8,105,447 B2**  
(45) **Date of Patent:** **Jan. 31, 2012**

(54) **AUSTENITIC STAINLESS HOT-ROLLED STEEL MATERIAL WITH EXCELLENT CORROSION RESISTANCE, PROOF STRESS, AND LOW-TEMPERATURE TOUGHNESS**

(75) Inventors: **Yuusuke Oikawa**, Tokyo (JP); **Shinji Tsuge**, Tokyo (JP); **Shigeo Fukumoto**, Tokyo (JP); **Kazuhiko Suetsugu**, Tokyo (JP); **Ryo Matsuhashi**, Chiba-ken (JP); **Hiroshige Inoue**, Chiba-ken (JP)

(73) Assignee: **Nippon Steel & Sumikin Stainless Steel Corporation**, Tokyo (JP)

(\*) Notice: Subject to any disclaimer, the term of this patent is extended or adjusted under 35 U.S.C. 154(b) by 279 days.

(21) Appl. No.: **12/391,045**

(22) Filed: **Feb. 23, 2009**

(65) **Prior Publication Data**

US 2010/0230011 A1 Sep. 16, 2010

**Related U.S. Application Data**

(63) Continuation of application No. 11/343,516, filed on Jan. 30, 2006, now abandoned.

(30) **Foreign Application Priority Data**

Feb. 2, 2005 (JP) ..... P 2005-026176  
Feb. 2, 2005 (JP) ..... P 2005-026177  
Jan. 20, 2006 (JP) ..... P 2006-012569

(51) **Int. Cl.**

*C22C 38/44* (2006.01)  
*C22C 30/00* (2006.01)  
*C22C 38/42* (2006.01)  
*C22C 38/48* (2006.01)  
*C22C 38/50* (2006.01)  
*C22C 38/54* (2006.01)

(52) **U.S. Cl.** ..... **148/327; 148/442; 420/43; 420/52; 420/53; 420/47; 420/586.1**

(58) **Field of Classification Search** ..... **420/52, 420/53, 43, 47, 586.1; 148/327, 608, 609, 148/546-548, 442**

See application file for complete search history.

(56) **References Cited**

**U.S. PATENT DOCUMENTS**

|                |         |                           |
|----------------|---------|---------------------------|
| 4,302,247 A    | 11/1981 | Abe et al.                |
| 4,341,555 A    | 7/1982  | Douthett et al.           |
| 4,675,156 A    | 6/1987  | Sakamoto et al.           |
| 6,576,068 B2 * | 6/2003  | Grubb et al. .... 148/327 |
| 6,918,968 B2   | 7/2005  | Semba et al.              |

**FOREIGN PATENT DOCUMENTS**

|              |         |
|--------------|---------|
| JP 59-006359 | 1/1984  |
| JP 60208459  | 10/1985 |
| JP 02097649  | 4/1990  |
| JP 04006214  | 1/1992  |
| JP 04006215  | 1/1992  |
| JP 04006216  | 1/1992  |

**OTHER PUBLICATIONS**

English—hand translation of Japanese patent No. 359006359, Oomura, Sadafumi et al., Jan. 13, 1984.\*

\* cited by examiner

*Primary Examiner* — Deborah Yee

(74) *Attorney, Agent, or Firm* — Dorsey & Whitney LLP

(57) **ABSTRACT**

An austenitic stainless steel hot-rolled steel material can be provided which has sea-water resistance and strength superior to conventional steel. Low-temperature toughness can be maintained, which is preferable in a structural member of speedy craft. The steel material can include an austenitic stainless steel hot-rolled steel material which excels in the properties of corrosion resistance, proof stress, and low-temperature toughness. In such austenitic stainless steel hot-rolling steel material, e.g.,  $\text{PI} [= \text{Cr} + 3.3(\text{Mo} + 0.5\text{W}) + 16\text{N}]$  ranges from 35 to 40,  $\delta_{\text{cal}} [= 2.9(\text{Cr} + 0.3\text{Si} + \text{Mo} + 0.5\text{W}) - 2.6(\text{Ni} + 0.3\text{Mn} + 0.25\text{Cu} + 35\text{C} + 20\text{N}) - 18]$  ranges from -6 to +2, and a 0.2% proof stress at room temperature is not less than 550 MPa, Charpy impact value measured using a V-notch test piece at -40° C. is not less than 100 J/cm<sup>2</sup>, and the pitting potential measured in a deaerated aqueous solution of 10% NaCl at 50° C. (V<sub>c</sub>100) is not less than 500 mV (as it relates to saturated Ag/AgCl).

**6 Claims, No Drawings**

## 1

**AUSTENITIC STAINLESS HOT-ROLLED  
STEEL MATERIAL WITH EXCELLENT  
CORROSION RESISTANCE, PROOF STRESS,  
AND LOW-TEMPERATURE TOUGHNESS**

**CROSS REFERENCE TO RELATED  
APPLICATION(S)**

This application is a continuation of U.S. Non-Provisional application Ser. No. 11/343,516 filed Jan. 30, 2006, now abandoned which claims priority under 35 U.S.C. §119 from Japanese Patent Application No. P2005-026176 and P2005-026177, both filed Feb. 2, 2005 and Japanese Patent Application No. 2006-012569, filed Jan. 20, 2006, the entire disclosures of which are incorporated herein by reference.

**FIELD OF THE INVENTION**

The present invention relates to a structural steel material which excels in corrosion resistance, and can be used in a marine (chloride) environment, for example; an austenite-type stainless steel hot-rolling steel material, as a hull-structural material which excels in strength as well as seawater resistance, and low-temperature toughness, upon being used as a material for an outer shell, a bulkhead, a frame, a hydrofoil, etc. The present invention also relate to a method for producing such steel material.

**BACKGROUND INFORMATION**

Conventionally, coated steel sheets to which a heavy corrosive protection was applied were used for hull structures. The demand for speedy craft equipped with hydrofoils etc. has increased. Since high-speed sea water flow can come into contact with the hydrofoils, etc., such use prefers the use of a material which excels in sea water resistance without requiring being coated. In order to reduce hull weight thither, a material having a high strength is preferred.

Although austenitic stainless steel can be important as a material which excels in sea water resistance, in a conventional production method, austenitic stainless steel is generally subjected to a solution annealing treatment after hot-rolling, thereby softening the resultant austenitic stainless steel so that the proof stress of the austenitic stainless steel is at most 400 MPa.

The strength can be increased by performing a hot-rolling processing under a specific temperature condition while omitting the solution annealing treatment, which has been described in Japanese Unexamined Patent Application, First Publication Nos. S. 60-208459, H. 2-97649, and H. 4-6214.

In particular, Japanese Unexamined Patent Application, First Publication No. H. 2-97649 describes a production method of an austenitic stainless steel having a high proof stress while maintaining a low-temperature toughness. However, the sea water resistance is not taken into consideration in this austenitic stainless steel while maintaining low-temperature toughness. Although Japanese Unexamined Patent Application, First Publication No. H. 4-6214 describes a production method of an austenitic stainless steel which has a high proof stress of not less than 500 MPa and excellent sea-water resistance, which includes performing a heat treatment on steel which contains 0.3% or more of N and 0.5 to 3.0% of Mo under a specific condition, there is no disclosure in this publication regarding the toughness of the material.

The official reports for Japanese Patent Publication Nos. 2783895 and 2783896 describe a production technique of an austenitic stainless steel with little softening of a weld part by adding a Nb-type element.

## 2

Cr, Mo, and N are elements which increase sea water resistance, and the corrosion resistance ranking in steel is determined by the formula:  $PI=Cr+3.3(Mo+0.5W)+16N$  as a pitting index. When the PI value of the component shown in examples of Japanese Unexamined Patent Application, First Publication No. H. 4-6214 is determined, it is approximately 32 in the minimum case, but as a stainless steel which gives a higher PI value (not less than 35), SUS36L and 890L (which contain 23% or more of Ni) are austenitic types, whereas 10 SUS329J4L (which contains 5.5 to 7.5% of Ni) is a two-phase type.

Since two-phase-type SUS329J4L contains a ferrite phase, SUS329J4L has high proof stress. A two-phase stainless steel known as a super two-phase, in which Mo and W contents are increased has also been developed, and application thereof as a material with high hardness and high corrosion resistance has started. On the other hand, a high strength steel material of an austenitic-type high corrosion resistance stainless steel having a PI value over 35 has not yet been put in practical use.

15 Stainless steel is more susceptible to crevice corrosion when it is shaped into a crevice form than when it is not shaped i.e. flat. Therefore, in order to produce steel suitable for broad use in hull structures and which is low-maintenance, it is required to develop a highly corrosion-resistant steel material which is higher than the steel material described in Japanese Unexamined Patent Application, First Publication No. H. 4-6214.

On the other hand, the demand for a stainless steel material for ocean-going craft which is reliable when stranded or after 20 a collision between shipping is increasing. Characteristics of both the base material and the weldability are preferred for reliability. Regarding the reliability of the base material, high toughness is preferred in preparation for a collision. Among Cr, Mo and N, which increase corrosion resistance, as for Mo and Cr, it may not be sufficient to simply add, because processability in hot-rolling will significantly decrease likely due to the influence of delta ferrite contained in cast steel or semi-finished products. In addition, in the case of a high Cr and Mo steel, in general, the toughness of the steel deteriorates 25 remarkably due to the influence of an intermetallic compound known as a  $\sigma$  phase, and hence it is necessary to add a large amount of Ni in order to suppress the influence of both. However, considering the rising prices of raw materials of Ni and Mo these days, development of a low-cost, highly corrosion-resistant stainless steel is especially desired. It should be noted that, two-phase steel may not be adopted because of its 30 low-temperature toughness.

On the other hand, as for adding N as described in Japanese Unexamined Patent Application, First Publication No. H. 4-6214, it may be effective for maintaining the strength, however, excessive N causes the generation of bubbles at a welded part, thereby it may decrease the bonding strength and reliability of the welded part, to the contrary.

Thus, it is one of the objects of the present invention to 35 provide an austenitic stainless steel hot-rolled steel material which has sea-water resistance and strength superior to the conventional steel, while maintaining low-temperature toughness, which is required in a structural member of a high-speed ship. Another object of the present invention is to 40 provide an austenitic stainless steel hot-rolled steel material which excels in the properties of corrosion resistance, proof stress, and low-temperature toughness.

The strength, the toughness, and the corrosion resistance of a hot-rolled plate obtained by casting, heat-rolling processing 45 has been reviewed, and it has been determined that it may be preferable to provide a heat treatment of an austenitic component system in which the N amount is not more than 0.35%

in view of weldability and the PI value is not less than 35, in view of weldability. In particular, it has been determined that the toughness cannot be determined by only the Ni content, but is determined by the content of intermetallic compounds, which are contained in a steel material, having high Cr and Mo contents. The formation of a metallographic structure as such starts from the solidification of steel, in addition, the formation may be generated at any steps in hot-rolling processing. In particular, the influence of a chemical composition on a solidified structure has been investigated, and the influence of conditions on rough rolling of cast steel, homogenizing heat treatment, hot working, and heat treatment has been reviewed. As a result, it was determined to restrict the content of component elements the solidification structure and the metallographic structure of a steel material to obtain an austenitic stainless steel which can address the problems of the conventional technique and excels in corrosion resistance, toughness, strength, and hot processability, the solidification structure, the metallographic structure of a steel material, thereby completing the austenitic stainless steel of the present invention and the production method thereof.

#### SUMMARY OF EXEMPLARY EMBODIMENTS OF THE INVENTION

According to one exemplary embodiment of the present invention, an austenitic stainless hot-rolled steel material having excellent corrosion resistance, proof stress, and low-temperature toughness can be provided. Such steel material can include: about 0.001 to 0.03 mass % of C, about 0.1 to 1.5 mass % of Si, about 0.1 to 3.0 mass % of Mn, about 0.005 to 0.05 mass % of P, about 0.0001 to 0.003 mass % of S, about 15.0 to 21.0 mass % of Ni, about 22.0 to 28.0 mass % of Cr, about 1.5 to 3.5 mass % of Mo, about 0.15 to 0.35 mass % of N, and about 0.0005 to 0.007 mass % of O. The PI value can be expressed by the following: (1) ranges from about 35 to 40,  $\delta$  cal value expressed by the following and (2) ranges from about -6 to +2, the remnant consists of Fe and inevitable impurities, the content of intermetallic compounds contained in the steel material is not more than about 0.5 mass %, a 0.2% proof stress at room temperature is not less than about 550 MPa, the Charpy impact value measured using a V-notch test piece at about -40° C. is not less than about 100 J/cm<sup>2</sup>, and the pitting potential measured in a deaerated aqueous solution of about 10% NaCl at 50° C. (Vc100) is not less than about 500 mV (vs saturated Ag/AgCl).

$$PI=Cr+3.3(Mo+0.5W)+16N \quad (1)$$

$$\delta \text{ cal}=2.9(Cr+0.3Si+Mo+0.5W)-2.6(Ni+0.3Mn+0.25Cu+35C+20N)-18 \quad (2)$$

In addition, according to further exemplary embodiments of the present invention, the following one or more of certain metallic elements can be included:

- a) one or more of about 0.3 to 3.0 mass % of W and about 0.005 to 0.1 mass % of Al.
- b) one or more of about 0.3 to 3.0 mass % of W, about 0.005 to 0.1 mass % of Al, about 0.3 to 2.0 mass % of Cu, and not more than about 0.1 mass % of Sn.
- c) one or more of about 0.3 to 3.0 mass % of W, about 0.005 to 0.1 mass % of Al, about 0.0005 to 0.0050 mass % of Ca, about 0.0005 to 0.0050 mass % of Mg, and about 0.005 to 0.10 mass % of REM.
- d) one or more of about 0.3 to 3.0 mass % of W, about 0.005 to 0.1 mass % of Al, about 0.0005 to 0.0050 mass % of Ca, about 0.0005 to 0.0050 mass % of Mg, about 0.005 to 0.10 mass % of REM, and about 0.0003 to 0.0060 mass % of B.

5) one or more of about 0.3 to 3.0 mass % of W, about 0.005 to 0.1 mass % of Al, about 0.3 to 2.0 mass % of Cu, not more than about 0.1 mass % of Sn, about 0.0005 to 0.0050 mass % of Ca, about 0.0005 to 0.0050 mass % of Mg, about 0.005 to 0.10 mass % of REM, about 0.0003 to 0.0060 mass % of B, about 0.003 to 0.03 mass % of Ti, about 0.02 to 0.20 mass % of Nb, about 0.003 to 0.03 mass % of Zr, about 0.05 to 0.5 mass % of V, and about 0.01 to 0.1 mass % of Ta.

According to still another exemplary embodiment of the present invention, a process can be provided for producing an austenitic stainless hot-rolled steel material having excellent corrosion resistance, proof stress, and low-temperature toughness, including: performing homogenizing-heat treatment on a cast steel or a semi-finished product of the austenitic stainless as described for the exemplary embodiments of the steel material above. This process can be performed at a temperature of about 1200 to 1300° C. for about 1 hour or more, reheating it at a temperature of about 1100 to 1300° C., rolling it by a draft of not less than 50% at a temperature of not lower than about 1050° C. and a draft of not less than about 10% at a temperature of about 1050 to 850° C., while maintaining a temperature of not lower than 850° C. in the rolling step, allowing an average cooling rate at about 800 to 500° C. after the rolling to be not less than about 150° C./min, and 20 performing no solution treatment.

Exemplary embodiments of the present invention can provide austenitic stainless steel having excellent sea water resistance, proof stress, and low-temperature toughness, by restricting the component and performing a specific heat treatment processing. An austenitic stainless steel can be obtained which may be suitable for hull structures having a high level of sea water resistance and proof stress and low-temperature toughness, which are required as components for structures of high-speed ships, and contributes to industry 30 significantly.

In a further exemplary embodiment of the present invention, an austenitic stainless hot-rolled steel material can be provided which has excellent corrosion resistance, and low-temperature toughness, including: not more than about 0.03 mass % of C, about 0.1 to 1.5 mass % of Si, about 0.1 to 3.0 mass % of Mn, not more than about 0.05 mass % of P, not more than about 0.003 mass % of S, about 15.0 to 21.0 mass % of Ni, about 22.0 to 28.0 mass % of Cr, about 1.5 to 3.5 mass % of Mo, about 0.15 to 0.35 mass % of N, about 0.005 to 0.1 mass % of Al, and not more than about 0.007 mass % of O, in which the PI value expressed by the following formula 40 (1) ranges from about 35 to 40,  $\delta$  cal value expressed by the following formula (2) ranges from about -6 to +4, the remnant consists of Fe and substantially inevitable impurities, and the content of intermetallic compounds contained in the steel material is not more than about 0.5 mass %,

$$PI=Cr+3.3(Mo+0.5W)+16N \quad (1)$$

$$\delta \text{ cal}=2.9(Cr+0.3Si+Mo+0.5W)-2.6(Ni+0.3Mn+0.25Cu+35C+20N)-18 \quad (2)$$

in which the value by each element represents the content of the element expressed in terms of mass %.

According to still another exemplary embodiment of the present invention, the austenitic stainless hot-rolled steel material having excellent corrosion resistance can be provided, and the low-temperature toughness, as described above for other exemplary embodiments of the present invention, and further including one or more selected from the group consisting of about 0.1 to 2.0 mass % of Cu, about 0.003 to 0.03 mass % of Ti, about 0.02 to 0.20 mass % of Nb, about 0.05 to 0.5 mass % of V, about 0.3 to 3.0 mass % of W, about 0.0003

to 0.0060 mass % of B, about 0.0005 to 0.0050 mass % of Ca, about 0.0005 to 0.0050 mass % of Mg, and about 0.005 to 0.10 of REM.

According to yet another exemplary embodiment of the present invention, a process can be provided for producing the austenitic stainless hot-rolled steel material having excellent corrosion resistance, and low-temperature toughness, as set forth in the eighth or ninth aspect of the present invention, including: performing homogenizing-heat treatment on a cast steel or a semi-finished product after a rough heat-rolling processing at a temperature of 1 about 200 to 1300° C. for 1 hour or more, in order to reduce the content of the intermetallic compound in the steel material.

Exemplary embodiments of the present invention are capable of providing an austenitic stainless steel suitable for hull structures having a high level of sea water resistance and proof stress, which are preferred as components for structures of high-speed ships, and low-temperature toughness, and provides a contribution to the industry.

These and other objects, features and advantages of the present invention will become apparent upon reading the following detailed description of embodiments of the invention, when taken in conjunction with the appended claims.

#### DETAILED DESCRIPTION OF EXEMPLARY EMBODIMENTS OF THE INVENTION

A first exemplary embodiment of the present invention is below. As an initial matter, the characteristics preferred for structural shipping materials are described as follows. For a corrosion resistance, it is preferable to withstand sea water even without a heavy duty corrosion-resistant coating being applied thereto, and those characteristics which may be preferable to satisfy such corrosion resistance can be investigated to obtain the following results.

For example, although a usual pitting electric potential is measured in 30° C.-3.5% NaCl, the water temperature often reaches 50° C., in consideration of sea water resistance in the tropics, and further, sea water is often condensed in a gappy structure so that the NaCl concentration may increase to be higher than the 3.5% of normal sea water, and it was revealed that if the pitting electrical potential (Vc'100) measured in a deaerated 50° C.-10% NaCl aqueous solution is not less than 500 mV, then there are no significant problems in terms of practical use. Saturated Ag/AgCl can be used as a reference electrode.

With respect to the impact resistance, since it becomes problematic conversely in cold areas, it can be specified that a Charpy impact value should be not less than 100 J/cm<sup>2</sup> at -40° C., at which it can be recognized in general that no problems occur in ships.

As for hardness, it is preferably to reduce the weight. Exemplary embodiments of the present invention can provide a steel material having a high strength with a 0.2% proof stress of not less than 550 MPa at room temperature, provided that the above corrosion resistance and the impact strength are satisfied.

Further, the reason for restricting the components in the present invention are as follows. For example, the content of C can be restricted to not more than 0.03%, in order to maintain the corrosion resistance of stainless steel. If the content of C exceeds 0.03%, then Cr carbide may be generated and corrosion resistance and toughness can deteriorate. However, if the content of C is significantly reduced, then the cost for refining increases, and hence the lower limit can be specified as 0.001% (e.g., preferably, 0.01 to 0.03%).

Si may be added at not less than 0.1% for deoxidation. However, if the content of Si exceeds 1.5%, then toughness may deteriorate. Therefore, the upper limit can be specified as 1.5% (e.g., preferably 0.2 to 1.0%).

5 Mn is added at not less than 0.1% for deoxidation. However, if the content of Mn exceeds 3.0%, then corrosion resistance and toughness will deteriorate. Therefore, the lower limit is specified as 3.0% (e.g., preferably 0.2 to 1.5%).

P can be provided at most 0.05%, because P deteriorates 10 the hot-rolling processability and toughness. However, if the content of P is remarkably decreased, then refining cost increases, and hence the lower limit is specified as 0.005% (e.g., preferably 0.01 to 0.03%).

S can be at most 0.003%, because S deteriorates the hot- 15 rolling processability, toughness, and corrosion resistance. However, if the content of S is remarkably decreased, then refining cost increases, and hence the lower limit is specified as 0.0001% (e.g., preferably 0.0005 to 0.001%).

Since Ni stabilizes an austenitic configuration, and 20 improves the corrosion resistance against various acids and toughness further, Ni is can be added at not less than about 15.0%. On the other hand, since Ni is an expensive metal, the content of Ni is restricted to not more than 21.0% from the viewpoint of cost.

25 Cr is contained at not less than about 22.0% in order to secure basic corrosion resistance. On the other hand, if Cr is contained at over 28.0%, then an intermetallic compound is likely to be deposited to deteriorate toughness. For this reason, the content of Cr is specified within a range of not less than 28.0% to not more than about 22.0%.

30 Mo is an effective element which raises the corrosion resistance of stainless steel additionally, and can be contained at not less than about 1.5% in the present invention. On the other hand, Mo is a very expensive element and Mo promotes deposition of an intermetallic compound with Cr, and hence the upper limit of Mo is specified as not more than 3.5%. Preferably the content of Mo ranges from 2.0 to 3.0%.

N is an effective element which intercrystallizes into an austenite phase to increase hardness and corrosion resistance. 40 For this reason, N is contained at not less than 0.15%. Although N can be intercrystallized into a base material by up to 0.4%, the upper limit of the content of N is specified as about 0.35%, because N raises the sensitivity of generation of bubbling when performing welding. Preferably, the content of N can be not more than about 0.30%.

45 O is an important element which constitutes an oxide which represents a nonmetallic inclusion, and excessive content of O deteriorates toughness, on the other hand, if a coarse cluster-like oxide is generated, then it cause surface cracking. For this reason, the upper limit of the content of O is restricted to 0.007%. Moreover, if the content of O is significantly decreased, then the cost for refining increases, and hence the lower limit is specified to about 0.0005%. Preferably, the content of O can range from 0.001 to 0.004%.

50 PI value can be expressed by the above formula (1). A pitting index may be an index of corrosion resistance of stainless steel to a chloride environment, and it was possible to obtain the preferred characteristics by providing the PI value to not less than 35. As stainless steel having a PI value of more than 40, SUS836L etc. are exemplary, but the content of Ni thereof is not less than 24%, and it is expensive. According to the exemplary embodiment of the present invention, since the target is an austenitic stainless steel which has corrosion resistance corresponding to cost, the upper limit of the PI value is specified as 40. It should be noted that, in the present invention which contains no W, the value of W in formula (1) can be set to 0.

The  $\delta_{\text{cal}}$  expressed by the above formula (2) may be an index which indicates the quantity of the delta ferrite which appears in the solidified configuration of austenitic stainless steel, and in order to reduce solidification crack sensitivity or to make a configuration fine, generally it is controlled to approximately 0 to 7%. However, in steel having a high content of Cr as in the present invention, delta ferrite in a solidified configuration changes into an intermetallic compound during the hot-rolling production step, and remains in a steel material as a by-product, thereby deteriorating toughness. For this reason, the upper limit of  $\delta_{\text{cal}}$  is restricted to +2 so that delta ferrite might decrease. If  $\delta_{\text{cal}}$  exceeds this value, then it becomes difficult to obtain high toughness even when devising in the hot-rolling production step. On the other hand, the side in which  $\delta_{\text{cal}}$  is small (minus) can mean that the delta ferrite content becomes substantially 0%. As a result, the above described effect is saturated and an excess of Ni content will be contained, and hence the lower limit is restricted to -6, in view of cost. Preferably,  $\delta_{\text{cal}}$  ranges from -3 to +1. It should be noted that in the present invention without containing W and Cu, the value of W or Cu in formula (2) is set to 0.

The content of intermetallic compound which is contained in steel materials is an important factor which dictates the toughness of the austenitic stainless steel material in the exemplary embodiment of the present invention. An intermetallic compound is a compound which contains Cr, Mo, or W, as main ingredients and is known as  $\sigma$  phase and  $\chi$  phase. The content of this compound can be measured by performing alkali electrolytic etching of the micro configuration and observing it with an approximately 400-power optical microscope. It has been determined that if this content as an average value of observation of the cross-section of a steel material exceeds 0.5%, then Charpy absorbed energy of the steel material becomes less than 100 J/cm<sup>2</sup>, and specified the upper limit thereof to be 0.5%.

The second exemplary embodiment of the present invention is described as follows.

W is an element which raises the corrosion resistance of stainless steel additionally as well as Mo, and W can be contained by an amount ranging from 0.3 to 3.0% in the exemplary embodiment of the present invention steel for this purpose.

Al is an important element for deoxidation of steel, and in order to reduce oxygen in steel, Al is contained by at amount of not less than 0.005%. On the other hand, Al is an element having a relatively large affinity to N, and hence if an excess of Al is added, then AlN is generated to deteriorate the toughness of stainless steel. Although the degree of deterioration of toughness depends on the N content, if the Al content exceeds 0.1%, then the toughness deteriorates significantly, and hence the upper limit of Al content is specified as 0.1%.

The third exemplary embodiment of the present invention is described as follows

Cu is an element which raises the corrosion resistance of stainless steel against an acid additionally, and Cu can be contained for this purpose. It is preferable to add Cu in an amount of not less than 0.3%, whereas if Cu in an amount of more than 2.0% is added, the effect in line with the cost is saturated, and hence the upper limit is specified as 2.0%.

Although Sn also raises the corrosion resistance of steel, an excess of Sn causes hot-rolling processing cracking, and hence the upper limit is specified as 0.1%. Preferably, the lower limit of Sn content is specified as 0.005%.

The fourth exemplary embodiment of the present invention is described as follows

Each of Ca, Mg, and REM(s) is an element which improves the hot-rolling processability of steel, and one or more of

them are added for this purpose. Excessive addition of each of them deteriorates the hot-rolling processability adversely, and hence the upper limit and the lower limit thereof are specified as follows. That is, the content of each of Ca and Mg ranges from 0.0005 to 0.0050%, and the content of REM ranges from 0.005 to 0.10%. Here, REM represents the total content of a lanthanide series rare-earth element such as La, Ce, etc.

Furthermore, the PV value specified by the following formula (3) is set to be not more than 0. This formula is one that clarifies the required amount Ca, Mg, and REM to be added based on the existing amount of S, and it is possible to add exactly by making the PV value to be not more than 0, thereby improving the hot-rolling processability further.

$$PV = S + O - 0.8Ca - 0.3Mg - 0.3REM - 30 \quad (3)$$

The fifth exemplary embodiment of the present invention is described as follows

As for B, by adding it in an amount of not less than 0.0003%, it becomes possible to increase grain boundary strength and improve the hot-rolling processability. However, since excessive addition of B deteriorates the hot-rolling processability to the contrary due to an excessively deposited boride, the upper limit of the B content is specified as 0.0060%.

The sixth exemplary embodiment of the present invention is described as follows

Ti is an element which forms an oxide, a nitride, and sulfide with a very small amount thereof, and makes the crystal grain of steel fine, and Ti is an element which can be advantageously used in the steel material of the present invention. In order to reduce the intermetallic compound content in steel materials, it is effective to restrict the upper limit value of  $\delta_{\text{cal}}$  and perform homogenizing heat treatment of semi-finished products. Among these, in the latter method, heat treatment at a high temperature of approximately 1250° C. can be performed for several hours, if a proper amount of Ti is contained therein, then growth of crystal grain during the heat treatment at a high temperature as such can be effectively suppressed. For this purpose, it is necessary to add Ti in an amount of not less than 0.003%. On the other hand, Ti is an element which has a high nitride-forming power, and hence if Ti in an amount of over 0.03% is contained in the steel material of the present invention which contains N, then coarse TiN will deteriorate the toughness of the steel. For this reason, Ti content is specified in the range of 0.003 to 0.03%. Preferably, the Ti content can have a range from 0.005 to 0.02%, in the case in which Ti is contained.

Nb forms carbide to fix C, thereby suppressing formation of Cr carbide to increase corrosion resistance and toughness. In addition, Nb forms nitride to suppress the growth of crystal grain, thereby converting steel material into fine grains to increase the strength. For improving corrosion resistance and increasing strength, Nb in an amount of not less than 0.02% can be contained. However, if Nb in an amount of over 0.2% is added, then a large amount of carbon nitride of Nb is deposited during the hot-rolling processing step to deteriorate the hot-rolling recrystallization and a coarse configuration will remain in a steel material as a product, and hence the upper limit of Nb content is specified as 0.2%. Preferably Nb content can have a range from 0.05% to 0.15%.

V is an element that forms a carbon nitride as well as Nb, and V can be added in order to maintain corrosion resistance and toughness. Although V is contained in an amount of not less than 0.05% for this purpose, if V in an amount of over 0.5% is contained, then a coarse V series carbon nitride will

be generated, and toughness will deteriorate conversely. Therefore, the upper limit of V is restricted to 0.5% (e.g., preferably from 0.1 to 0.3%).

Although Zr and Ta can inhibit the negative influence on the corrosion resistance of C or S by addition, if Zr or Ta is added excessively, then deterioration of toughness will occur, and hence Zr content is restricted to 0.003 to 0.03% and Ta content can be provided at 0.01 to 0.1%.

The seventh exemplary embodiment of the present invention is described as follows

In order to increase the toughness of steel materials in the present invention, the amount of intermetallic compound contained in the steel material is restricted to not more than 0.5%, however, solidifying heat treatment after the final heat-rolling step must be omitted in order to obtain high proof stress. Therefore, as for an intermetallic compound, it is necessary to reduce the intermetallic compound contained in a cast steel, and to prevent formation of the intermetallic compound during the hot-rolling step as far as possible.

First, as the technique for reducing the intermetallic compound in the cast steel, it is preferable to combine the controlling of  $\delta$  cal with the homogenizing heat treatment to the cast steel of steel described in this exemplary embodiment. In the case in which there is no solidification segregation in the target steel materials of the present invention, the temperature at which an intermetallic compound is generated is approximately not higher than 1000°C. However, in the semi-finished product which is accompanied with segregation of ingredients caused by solidification, it becomes necessary to perform a production step for diffusing the segregation and homogenizing it in order to reduce the content of an intermetallic compound in the semi-finished product. Although the temperature and the time of this homogenizing heat treatment can change slightly, corresponding to chemical composition such as solidifying rate and cross-sectional area of the cast steel, the degree of hot-rolling processing when processing into a semi-finished product, and  $\delta$  cal, etc., the temperature required is not lower than 1200°C., because the rate is limited by diffusion of Cr, Mo, Ni, etc. On the other hand, if the temperature exceeds 1300°C., then oxidized scale may be generated more than usually. As for the time, it is preferable that the time be as long as possible, and at least one hour is necessary. Moreover, this purpose can be attained by performing a soaking at 1200°C. for one hour or more during heating of the semi-finished product for rolling a product. As mentioned above, it is specified to perform homogenizing heat treatment for one hour or more at a temperature ranging from 1200 to 1300°C. Taking the effect and the economical efficiency into consideration, a preferable range of soaking time ranges from 2 to 20 hours.

As for the rolling condition, it consists of the rough rolling stage in which re-heating is performed at a temperature ranging from 1100 to 1300°C. and making the total compaction amount at a temperature of not lower than 1050°C. to be not less than 50%, and the successive finishing rolling stage in which the total compaction amount at a temperature ranging from 1050 to 850°C. is made to be not less than 10%. The rough rolling stage is a stage in which the solidification structure is mainly destroyed, to obtain a uniform recrystallized

structure, whereas the finishing rolling step is a step of introducing the processing strain by the rolling and for increasing the strength after the rolling processing. In addition, all of the rolling processing is performed at a temperature of not lower than 850°C., thereby preventing the re-deposition of the intermetallic compound. Further, a controlled cooling is performed at an average cooling rate of not less than 150°C./min from 800 to 500°C. after the rolling processing, thereby inhibiting the re-deposition of the intermetallic compound and the recovery of the processing strain which was introduced in the finishing rolling step.

The exemplary reason for restricting the condition is described in further detail below. In order to make it possible to perform a rolling processing which makes the total compaction amount to be not less than 50% at a temperature of not lower than 1050°C., to reduce deformation resistance, and to make it easy to perform the rolling processing, it is necessary to heat the steel ingot to not lower than 1100°C. However, if it is heated over 1300°C., then the grain boundary will be fused to cause cracks during the hot-rolled processing, and hence the heating temperature is restricted to be within a range of 1100 to 1300°C.

In the rough rolling stage, in order to destroy the solidification structure and to obtain a uniform recrystallized structure, it is necessary to make the total compaction amount at a temperature of not lower than 1050°C. to be not less than 50%. If the rolling temperature is lower than 1050°C. or the total compaction amount is less than 50%, then it is not possible to obtain uniform recrystallized structure.

In the finishing rolling stage, in order to acquire the target proof stress of 550 MPa, it is necessary to perform a finishing rolling by which the total compaction amount at a temperature of 1050°C. to 850°C. in the component range which is restricted in the present invention should be not less than 10%. In addition, if a rolling processing is performed at a temperature over 1050°C., then recrystallization will occur, and as a result compressing strain cannot be accumulated, so that sufficient strength cannot be obtained, whereas if a rolling processing is performed at a temperature lower than 850°C., then deposition of the intermetallic compound will be promoted to deteriorate toughness remarkably. Therefore, it is preferable to perform the rolling processing during all of the rolling processing, while maintaining the temperature to be not lower than 850°C. Finally, high hardness can be maintained by omitting solution heat treatment.

#### EXAMPLE 1

The chemical constitution of a test piece of steel is shown in Table 1. It should be noted that, the content of inevitable impurity elements other than the components indicated in Table 1 is the same level as in standard stainless steel. Moreover, as to the portions where no contents are shown for the components shown in Table 1, this means that the content is the same level as in an impurity level. Moreover, REM in the Tables represents lanthanoid series rare earth elements, and the content indicates the total of these elements. These steel samples were melted in a 50 kg-vacuum induction furnace in a laboratory and cast into a flat steel ingot having a thickness of approximately 100 mm.

TABLE 1-1

| STEEL No. | C         | Si    | Mn   | P    | S     | Ni     | Cr    | Mo    | Cu   |      |
|-----------|-----------|-------|------|------|-------|--------|-------|-------|------|------|
| A         | EXAMPLE 1 | 0.021 | 0.49 | 0.48 | 0.020 | 0.0005 | 17.91 | 25.15 | 2.31 | 0.12 |
| B         | EXAMPLE 1 | 0.019 | 0.46 | 0.32 | 0.023 | 0.0003 | 18.23 | 24.65 | 2.45 | 0.21 |
| C         | EXAMPLE 2 | 0.018 | 0.52 | 0.52 | 0.014 | 0.0005 | 17.98 | 25.02 | 2.46 | 0.05 |

TABLE 1-1-continued

| STEEL No. |             | C            | Si          | Mn          | P            | S             | Ni           | Cr           | Mo          | Cu   |
|-----------|-------------|--------------|-------------|-------------|--------------|---------------|--------------|--------------|-------------|------|
| D         | EXAMPLE 3   | 0.022        | 0.49        | 0.52        | 0.022        | 0.0006        | 18.43        | 24.88        | 2.46        | 0.45 |
| E         | EXAMPLE 3   | 0.015        | 0.71        | 1.71        | 0.026        | 0.0002        | 19.25        | 26.35        | 1.92        | 0.22 |
| F         | EXAMPLE 4   | 0.021        | 0.48        | 0.52        | 0.022        | 0.0009        | 18.25        | 25.36        | 2.53        | 0.30 |
| G         | EXAMPLE 4   | 0.022        | 0.46        | 0.52        | 0.021        | 0.0008        | 20.21        | 24.96        | 2.46        | 0.31 |
| H         | EXAMPLE 4   | 0.022        | 0.48        | 0.49        | 0.022        | 0.0003        | 19.23        | 24.64        | 3.33        | 0.28 |
| I         | EXAMPLE 5   | 0.021        | 0.47        | 0.52        | 0.022        | 0.0007        | 18.33        | 24.66        | 2.48        | 0.32 |
| J         | EXAMPLE 6   | 0.019        | 0.45        | 0.53        | 0.023        | 0.0008        | 18.23        | 24.65        | 2.46        | 0.32 |
| K         | EXAMPLE 6   | 0.019        | 0.49        | 0.49        | 0.022        | 0.0004        | 20.42        | 27.31        | 1.68        | 0.31 |
| L         | EXAMPLE 6   | 0.024        | 0.49        | 0.49        | 0.021        | 0.0003        | 19.53        | 24.61        | 2.11        | 1.82 |
| M         | EXAMPLE 6   | 0.019        | 0.49        | 0.85        | 0.019        | 0.0013        | 18.89        | 25.29        | 2.52        | 0.32 |
| N         | EXAMPLE 6   | 0.021        | 0.50        | 0.84        | 0.019        | 0.0005        | 16.77        | 25.21        | 2.10        | 0.85 |
| a         | COMPARATIVE | <u>0.035</u> | 0.35        | 0.25        | 0.008        | 0.0009        | 17.91        | 24.68        | 2.35        | 0.21 |
|           | EXAMPLE     |              |             |             |              |               |              |              |             |      |
| b         | COMPARATIVE | 0.006        | <u>1.75</u> | 2.11        | 0.027        | 0.0006        | 18.93        | 24.67        | 2.64        | 0.06 |
| c         | COMPARATIVE | 0.025        | 0.44        | <u>3.31</u> | 0.018        | 0.0010        | 17.59        | 27.19        | 1.65        | 0.58 |
|           | EXAMPLE     |              |             |             |              |               |              |              |             |      |
| d         | COMPARATIVE | 0.018        | 0.51        | 0.51        | <u>0.055</u> | 0.0003        | 18.21        | 23.77        | 2.33        | 0.91 |
|           | EXAMPLE     |              |             |             |              |               |              |              |             |      |
| e         | COMPARATIVE | 0.017        | 0.40        | 0.55        | 0.012        | <u>0.0033</u> | 17.64        | 24.21        | 2.58        | 1.22 |
|           | EXAMPLE     |              |             |             |              |               |              |              |             |      |
| f         | COMPARATIVE | 0.022        | 0.36        | 0.61        | 0.026        | 0.0008        | <u>14.55</u> | 22.91        | 2.53        | 0.46 |
|           | EXAMPLE     |              |             |             |              |               |              |              |             |      |
| g         | COMPARATIVE | 0.008        | 0.33        | 1.21        | 0.013        | 0.0006        | 20.12        | 27.55        | <u>1.22</u> | 0.25 |
|           | EXAMPLE     |              |             |             |              |               |              |              |             |      |
| h         | COMPARATIVE | 0.028        | 0.53        | 0.43        | 0.022        | 0.0006        | 18.88        | 22.84        | <u>3.68</u> | 0.66 |
|           | EXAMPLE     |              |             |             |              |               |              |              |             |      |
| i         | COMPARATIVE | 0.033        | 0.15        | 0.35        | 0.026        | 0.0004        | 20.55        | 25.35        | 2.33        | 0.24 |
|           | EXAMPLE     |              |             |             |              |               |              |              |             |      |
| j         | COMPARATIVE | 0.022        | 0.47        | 0.53        | 0.025        | 0.0008        | 18.21        | 24.96        | 2.46        | 0.33 |
|           | EXAMPLE     |              |             |             |              |               |              |              |             |      |
| k         | COMPARATIVE | 0.021        | 0.26        | 1.85        | 0.022        | 0.0009        | 15.61        | <u>21.89</u> | 2.12        | 0.31 |
|           | EXAMPLE     |              |             |             |              |               |              |              |             |      |
| l         | COMPARATIVE | 0.021        | 0.48        | 0.51        | 0.024        | 0.0007        | <u>18.55</u> | <u>28.22</u> | 2.01        | 0.31 |
|           | EXAMPLE     |              |             |             |              |               |              |              |             |      |
| m         | COMPARATIVE | 0.022        | 0.49        | 0.52        | 0.023        | 0.0008        | <u>21.40</u> | 24.95        | 2.47        | 0.33 |
|           | EXAMPLE     |              |             |             |              |               |              |              |             |      |
| n         | COMPARATIVE | 0.024        | 0.45        | 0.52        | 0.024        | 0.0006        | 18.22        | 24.94        | 2.47        | 0.31 |
|           | EXAMPLE     |              |             |             |              |               |              |              |             |      |
| o         | COMPARATIVE | 0.022        | 0.51        | 0.18        | 0.037        | 0.0028        | 19.56        | 25.61        | 2.64        | 0.35 |
|           | EXAMPLE     |              |             |             |              |               |              |              |             |      |
| p         | COMPARATIVE | 0.019        | 0.53        | 0.46        | 0.021        | 0.0003        | 18.36        | 24.91        | 2.28        | 0.36 |
|           | EXAMPLE     |              |             |             |              |               |              |              |             |      |
| q         | COMPARATIVE | 0.018        | 0.56        | 0.53        | 0.021        | 0.0006        | 16.95        | 22.21        | 3.39        | 1.66 |
|           | EXAMPLE     |              |             |             |              |               |              |              |             |      |
| r         | COMPARATIVE | 0.026        | 1.22        | 0.66        | 0.016        | 0.0003        | 17.91        | 23.96        | 2.31        | 0.33 |
|           | EXAMPLE     |              |             |             |              |               |              |              |             |      |
| s         | COMPARATIVE | 0.021        | 0.48        | 0.53        | 0.023        | 0.0008        | 18.23        | 24.89        | 2.46        | 0.32 |
|           | EXAMPLE     |              |             |             |              |               |              |              |             |      |
| t         | COMPARATIVE | 0.022        | 0.47        | 0.54        | 0.024        | 0.0007        | 18.33        | 23.33        | 2.45        | 0.35 |
|           | EXAMPLE     |              |             |             |              |               |              |              |             |      |
| u         | COMPARATIVE | 0.023        | 0.46        | 0.55        | 0.023        | 0.0008        | 18.25        | 24.98        | 2.48        | 0.32 |
|           | EXAMPLE     |              |             |             |              |               |              |              |             |      |
| v         | COMPARATIVE | 0.013        | 0.48        | 1.21        | 0.013        | 0.0005        | 16.36        | 22.64        | 2.93        | 0.28 |
|           | EXAMPLE     |              |             |             |              |               |              |              |             |      |
| w         | COMPARATIVE | 0.024        | 0.55        | 0.78        | 0.019        | 0.0005        | 17.21        | 23.51        | 2.33        | 0.33 |

—: VALUE WITHOUT THE RANGE OF THE PRESENT INVENTION

TABLE 1-2

| STEEL No. |           | Cu   | Sn   | Nb    | Ti    | V    | Zr | Te | W    | Al         |
|-----------|-----------|------|------|-------|-------|------|----|----|------|------------|
| A         | EXAMPLE 1 | 0.12 |      |       |       |      |    |    |      |            |
| B         | EXAMPLE 1 | 0.21 |      |       |       |      |    |    |      | 1.05       |
| C         | EXAMPLE 2 | 0.05 |      |       |       |      |    |    |      | 0.018      |
| D         | EXAMPLE 3 | 0.45 |      |       |       |      |    |    |      | 0.032      |
| E         | EXAMPLE 3 | 0.22 | 0.08 |       |       |      |    |    |      | 0.051      |
| F         | EXAMPLE 4 | 0.30 |      |       |       |      |    |    |      | 0.026      |
| G         | EXAMPLE 4 | 0.31 |      |       |       |      |    |    |      | 0.71 0.028 |
| H         | EXAMPLE 4 | 0.28 |      |       |       |      |    |    |      | 0.034      |
| I         | EXAMPLE 5 | 0.32 |      |       |       |      |    |    |      | 0.022      |
| J         | EXAMPLE 6 | 0.32 |      |       | 0.012 |      |    |    |      | 0.023      |
| K         | EXAMPLE 6 | 0.31 |      | 0.121 |       |      |    |    |      | 0.011      |
| L         | EXAMPLE 6 | 1.82 |      |       |       | 0.28 |    |    | 2.10 | 0.023      |

TABLE 1-2-continued

\_\_\_\_: VALUE WITHOUT THE RANGE OF THE PRESENT INVENTION

TABLE 1-3

| STEEL No. | B                      | Ca     | Mg     | REM   | O      | N     | δ cal | PI   | PV    |
|-----------|------------------------|--------|--------|-------|--------|-------|-------|------|-------|
| A         | EXAMPLE 1              |        |        |       | 0.0055 | 0.235 | 0.9   | 36.5 | 30.0  |
| B         | EXAMPLE 1              |        |        |       | 0.0063 | 0.266 | -0.8  | 38.8 | 36.0  |
| C         | EXAMPLE 2              |        |        |       | 0.0041 | 0.266 | -0.5  | 37.4 | 16.0  |
| D         | EXAMPLE 3              |        |        |       | 0.0025 | 0.240 | -1.4  | 36.8 | 1.0   |
| E         | EXAMPLE 3              |        |        |       | 0.0030 | 0.281 | -2.9  | 37.2 | 2.0   |
| F         | EXAMPLE 4              | 0.0022 |        |       | 0.0035 | 0.238 | 1.0   | 37.5 | -3.6  |
| G         | EXAMPLE 4              |        | 0.0033 |       | 0.0025 | 0.242 | -4.8  | 38.1 | -6.9  |
| H         | EXAMPLE 4              |        |        | 0.009 | 0.0019 | 0.257 | -2.4  | 39.7 | -35.0 |
| I         | EXAMPLE 5              | 0.0033 |        |       | 0.0026 | 0.235 | -1.3  | 36.6 | 3.0   |
| J         | EXAMPLE 6              | 0.0008 | 0.0033 |       | 0.0035 | 0.247 | -1.6  | 36.7 | -3.3  |
| K         | EXAMPLE 6              | 0.0023 |        |       | 0.0036 | 0.245 | -1.6  | 36.8 | -8.4  |
| L         | EXAMPLE 6              | 0.0020 |        |       | 0.0026 | 0.173 | -0.6  | 37.8 | -18.0 |
| M         | EXAMPLE 6              | 0.0008 |        | 0.021 | 0.0040 | 0.235 | -0.9  | 37.4 | -46.4 |
| N         | EXAMPLE 6              | 0.0042 |        |       | 0.0020 | 0.315 | -1.5  | 37.2 | -38.6 |
| a         | COMPARATIVE<br>EXAMPLE |        |        |       | 0.0022 | 0.193 | 0.6   | 35.5 | 1.0   |
| b         | COMPARATIVE<br>EXAMPLE | 0.0006 |        |       | 0.0034 | 0.264 | -2.5  | 37.6 | 5.2   |
| c         | COMPARATIVE<br>EXAMPLE | 0.0009 |        |       | 0.0022 | 0.252 | 1.9   | 36.7 | 2.0   |

TABLE 1-3-continued

| STEEL No. |                     | B             | Ca            | Mg            | REM          | O             | N            | $\delta$ cal | PI          | PV     |
|-----------|---------------------|---------------|---------------|---------------|--------------|---------------|--------------|--------------|-------------|--------|
| d         | COMPARATIVE EXAMPLE |               |               | 0.0008        |              | 0.0028        | 0.265        | -5.6         | 35.7        | -1.4   |
| e         | COMPARATIVE EXAMPLE |               | 0.0012        |               |              | 0.0009        | 0.237        | -0.9         | 36.5        | 2.4    |
| f         | COMPARATIVE EXAMPLE | 0.0028        |               | 0.0022        |              | 0.0026        | 0.279        | 1.0          | 35.7        | -2.6   |
| g         | COMPARATIVE EXAMPLE |               |               |               |              | 0.0026        | 0.295        | -3.8         | 36.3        | 2.0    |
| h         | COMPARATIVE EXAMPLE |               |               |               |              | 0.0034        | 0.155        | 0.9          | 39.7        | 10.0   |
| i         | COMPARATIVE EXAMPLE |               |               |               | 0.035        | 0.0052        | <u>0.121</u> | -0.8         | 35.0        | -79.0  |
| j         | COMPARATIVE EXAMPLE |               | 0.0036        |               |              | <u>0.0081</u> | 0.242        | -0.6         | 37.0        | 30.2   |
| k         | COMPARATIVE EXAMPLE |               | 0.0019        | 0.0008        |              | 0.0032        | 0.184        | -1.9         | <u>31.8</u> | -6.6   |
| l         | COMPARATIVE EXAMPLE |               | 0.0022        |               |              | 0.0029        | 0.271        | <u>5.3</u>   | 39.2        | -11.6  |
| m         | COMPARATIVE EXAMPLE |               | 0.0023        |               |              | 0.0030        | 0.240        | <u>-8.8</u>  | 36.9        | -10.4  |
| n         | COMPARATIVE EXAMPLE |               | 0.0024        |               |              | 0.0032        | 0.235        | -0.5         | 36.9        | -11.2  |
| o         | COMPARATIVE EXAMPLE |               | <u>0.0067</u> |               |              | 0.0032        | 0.222        | 0.5          | 38.9        | -23.6  |
| p         | COMPARATIVE EXAMPLE |               |               | <u>0.0071</u> |              | 0.0032        | 0.262        | -2.4         | 36.6        | -16.3  |
| q         | COMPARATIVE EXAMPLE |               | 0.0030        |               | <u>0.111</u> | 0.0032        | 0.212        | -1.5         | 36.8        | -349.0 |
| r         | COMPARATIVE EXAMPLE | <u>0.0071</u> |               |               |              | 0.0032        | 0.222        | -2.0         | 35.1        | 5.0    |
| s         | COMPARATIVE EXAMPLE |               | 0.0025        |               |              | 0.0032        | 0.241        | -0.7         | 36.9        | -10.0  |
| t         | COMPARATIVE EXAMPLE |               | 0.0026        |               | 0.015        | 0.0033        | 0.173        | -0.5         | 36.0        | -55.8  |
| u         | COMPARATIVE EXAMPLE |               | 0.0025        |               |              | 0.0031        | 0.239        | -0.6         | 37.0        | -11.0  |
| v         | COMPARATIVE EXAMPLE |               |               | 0.0025        |              | 0.0030        | 0.263        | -2.0         | 36.5        | -2.5   |
| w         | COMPARATIVE EXAMPLE |               |               |               |              | 0.0025        | 0.245        | -3.1         | 35.1        | 0.0    |

      : VALUE WITHOUT THE RANGE OF THE PRESENT INVENTION

A steel sheet having a thickness ranging from 12 to 22 mm was produced by performing cogging, homogenizing heat treatment, and product rolling, using the above sample steel. In the cogging, the sample steel was soaked at 1180° C. for two hours, and thereafter the sample steel was rolled to 65 mm thickness. Then the resultant semi-finished products were subjected to homogenizing heat treatment under the conditions shown in Tables 2 and 3. Some of the semi-finished products were not subjected to the homogenizing heat treatment. Each piece of steel was ground to 60 mm to obtain the

material for use in product rolling, and thereafter the resultant material for use in product rolling was subjected to hot-rolling processing to obtain a hot-rolled steel material. It should be noted that the steel material immediately after being hot-rolled which was in a temperature state of not less than 800° C. was cooled to a temperature of not higher than 500° C. by performing spray cooling. Some of the steel sheets were subjected to a solution heat treatment under the condition of 1100° C.×20 min with cooling by water, after soaking.

TABLE 2-1

| No. | STEEL No. | INTERMETALLIC COMPOUND CONTENT (%) | HOMOGENIZING HEAT TREATMENT | RE-HEATING TEMPERATURE (° C.) | REDUCTION AT 1050° C. OR MORE (%) | REDUCTION AT A TEMPERATURE OF 1050 TO 850° C. (%) |
|-----|-----------|------------------------------------|-----------------------------|-------------------------------|-----------------------------------|---------------------------------------------------|
| 1   | A         | EXAMPLE 0.35                       | 1250° C. × 4 h              | 1200                          | 60                                | 20                                                |
| 2   | B         | EXAMPLE 0.05                       | 1250° C. × 4 h              | 1200                          | 60                                | 20                                                |
| 3   | C         | EXAMPLE 0.10                       | 1250° C. × 4 h              | 1200                          | 60                                | 20                                                |
| 4   | D         | EXAMPLE 0.20                       | 1250° C. × 4 h              | 1200                          | 60                                | 20                                                |
| 5   | E         | EXAMPLE 0.05                       | 1250° C. × 4 h              | 1200                          | 60                                | 20                                                |
| 6   | F         | EXAMPLE 0.30                       | 1250° C. × 4 h              | 1200                          | 60                                | 20                                                |
| 7   | F         | EXAMPLE 0.35                       | 1220° C. × 2 h              | 1200                          | 60                                | 20                                                |
| 8   | F         | EXAMPLE 0.25                       | 1200° C. × 20 h             | 1200                          | 60                                | 20                                                |
| 9   | F         | EXAMPLE 0.40                       | 1250° C. × 4 h              | 1250                          | 60                                | 20                                                |
| 10  | F         | EXAMPLE 0.30                       | 1250° C. × 4 h              | 1200                          | 75                                | 15                                                |
| 11  | F         | EXAMPLE 0.30                       | 1250° C. × 4 h              | 1200                          | 60                                | 12                                                |
| 12  | F         | COMPARATIVE EXAMPLE 0.95           | <u>UNDONE</u>               | 1200                          | 60                                | 20                                                |
| 13  | F         | COMPARATIVE EXAMPLE 0.75           | <u>1150° C. × 5 h</u>       | 1200                          | 60                                | 20                                                |

TABLE 2-1-continued

| No. | STEEL No. |                     | INTERMETALLIC COMPOUND CONTENT (%) | HOMOGENIZING HEAT TREATMENT | RE-HEATING TEMPERATURE (° C.) | REDUCTION AT 1050° C. OR MORE (%) | REDUCTION AT A TEMPERATURE OF 1050 TO 850° C. (%) |
|-----|-----------|---------------------|------------------------------------|-----------------------------|-------------------------------|-----------------------------------|---------------------------------------------------|
| 14  | F         | COMPARATIVE EXAMPLE | <u>0.80</u>                        | <u>1200° C. x 15 m</u>      | 1200                          | 60                                | 20                                                |
| 15  | F         | COMPARATIVE EXAMPLE | 0.45                               | 1250° C. x 4 h              | <u>1050</u>                   | <u>0</u>                          | 68                                                |
| 16  | F         | COMPARATIVE EXAMPLE | 0.35                               | 1250° C. x 4 h              | 1200                          | 60                                | <u>7</u>                                          |
| 17  | F         | COMPARATIVE EXAMPLE | <u>0.60</u>                        | 1250° C. x 4 h              | 1200                          | 60                                | 20                                                |
| 18  | F         | COMPARATIVE EXAMPLE | <u>0.85</u>                        | 1250° C. x 4 h              | 1200                          | 60                                | 20                                                |
| 19  | F         | COMPARATIVE EXAMPLE | 0.00                               | 1250° C. x 4 h              | 1200                          | 60                                | 20                                                |
| 20  | G         | EXAMPLE             | 0.20                               | 1250° C. x 4 h              | 1200                          | 60                                | 5                                                 |
| 21  | H         | EXAMPLE             | 0.25                               | 1250° C. x 4 h              | 1200                          | 60                                | 20                                                |
| 22  | I         | EXAMPLE             | 0.30                               | 1250° C. x 4 h              | 1200                          | 60                                | 20                                                |
| 23  | J         | EXAMPLE             | 0.20                               | 1250° C. x 4 h              | 1200                          | 60                                | 20                                                |

—: VALUE WITHOUT THE RANGE OF THE PRESENT INVENTION

TABLE 2-2

| No. | STEEL No. |                     | ROLLING FINISHING TEMPERATURE (° C.) | COOLING RATE AT A TEMPERA-TURE OF 800 TO 500° C. (° C./min) | SOLUTION HEAT TREATMENT | EAR CRACK (mm) | PROOF STRESS (MPa) | vE-40° C. (J/cm <sup>2</sup> ) | Vc' 100 (mV vs Saturated Ag/AgCl) |
|-----|-----------|---------------------|--------------------------------------|-------------------------------------------------------------|-------------------------|----------------|--------------------|--------------------------------|-----------------------------------|
| 1   | A         | EXAMPLE             | 900                                  | 250                                                         | UNDONE                  | 5              | 710                | 130                            | 630                               |
| 2   | B         | EXAMPLE             | 900                                  | 250                                                         | UNDONE                  | 8              | 730                | 147                            | 750                               |
| 3   | C         | EXAMPLE             | 900                                  | 250                                                         | UNDONE                  | 5              | 726                | 187                            | 700                               |
| 4   | D         | EXAMPLE             | 900                                  | 250                                                         | UNDONE                  | 3              | 711                | 201                            | 685                               |
| 5   | E         | EXAMPLE             | 900                                  | 250                                                         | UNDONE                  | 5              | 733                | 203                            | 705                               |
| 6   | F         | EXAMPLE             | 900                                  | 250                                                         | UNDONE                  | 0              | 713                | 199                            | 720                               |
| 7   | F         | EXAMPLE             | 900                                  | 250                                                         | UNDONE                  | 0              | 720                | 167                            | 715                               |
| 8   | F         | EXAMPLE             | 900                                  | 250                                                         | UNDONE                  | 0              | 710                | 195                            | 720                               |
| 9   | F         | EXAMPLE             | 900                                  | 250                                                         | UNDONE                  | 0              | 706                | 163                            | 710                               |
| 10  | F         | EXAMPLE             | 900                                  | 250                                                         | UNDONE                  | 0              | 716                | 200                            | 710                               |
| 11  | F         | EXAMPLE             | 900                                  | 250                                                         | UNDONE                  | 0              | 590                | 225                            | 725                               |
| 12  | F         | COMPARATIVE EXAMPLE | 900                                  | 250                                                         | UNDONE                  | 0              | 729                | <u>63</u>                      | 625                               |
| 13  | F         | COMPARATIVE EXAMPLE | 900                                  | 250                                                         | UNDONE                  | 0              | 724                | <u>74</u>                      | 645                               |
| 14  | F         | COMPARATIVE EXAMPLE | 900                                  | 250                                                         | UNDONE                  | 0              | 725                | <u>66</u>                      | 630                               |
| 15  | F         | COMPARATIVE EXAMPLE | 900                                  | 250                                                         | UNDONE                  | 0              | 735                | <u>70</u>                      | 685                               |
| 16  | F         | COMPARATIVE EXAMPLE | 900                                  | 250                                                         | UNDONE                  | 0              | <u>538</u>         | 281                            | 730                               |
| 17  | F         | COMPARATIVE EXAMPLE | <u>800</u>                           | 250                                                         | UNDONE                  | 0              | 730                | <u>55</u>                      | 550                               |
| 18  | F         | COMPARATIVE EXAMPLE | 900                                  | <u>75</u>                                                   | UNDONE                  | 0              | 716                | <u>57</u>                      | 535                               |
| 19  | F         | COMPARATIVE EXAMPLE | 900                                  | 250                                                         | <u>DONE</u>             | 0              | <u>345</u>         | 350                            | 780                               |
| 20  | G         | EXAMPLE             | 900                                  | 250                                                         | UNDONE                  | 0              | 725                | 202                            | 740                               |
| 21  | H         | EXAMPLE             | 900                                  | 250                                                         | UNDONE                  | 0              | 724                | 217                            | 775                               |
| 22  | I         | EXAMPLE             | 900                                  | 250                                                         | UNDONE                  | 0              | 712                | 193                            | 645                               |
| 23  | J         | EXAMPLE             | 900                                  | 250                                                         | UNDONE                  | 0              | 729                | 164                            | 680                               |

—: VALUE WITHOUT THE RANGE OF THE PRESENT INVENTION

TABLE 3-1

| No. | STEEL No. |         | INTERMETALLIC COMPOUND CONTENT (%) | HOMOGENIZING HEAT TREATMENT | RE-HEATING TEMPERATURE (° C.) | REDUCTION AT 1050° C. OR MORE (%) | REDUCTION AT A TEMPERATURE OF 1050 TO 850° C. (%) |
|-----|-----------|---------|------------------------------------|-----------------------------|-------------------------------|-----------------------------------|---------------------------------------------------|
| 24  | K         | EXAMPLE | 0.15                               | 1250° C. x 4 h              | 1200                          | 60                                | 20                                                |
| 25  | K         | EXAMPLE | 0.20                               | 1250° C. x 4 h              | 1200                          | 60                                | 35                                                |
| 26  | K         | EXAMPLE | 0.30                               | 1250° C. x 4 h              | 1200                          | 60                                | 20                                                |
| 27  | K         | EXAMPLE | 0.05                               | 1250° C. x 4 h              | 1200                          | 60                                | 20                                                |
| 28  | K         | EXAMPLE | 0.05                               | 1250° C. x 4 h              | 1200                          | 60                                | 20                                                |

TABLE 3-1-continued

| No. | STEEL No. |                     | INTERMETALLIC COMPOUND CONTENT (%) | HOMOGENIZING HEAT TREATMENT | RE-HEATING TEMPERATURE (° C.) | REDUCTION AT 1050° C. OR MORE (%) | REDUCTION AT A TEMPERATURE OF 1050 TO 850° C. (%) |
|-----|-----------|---------------------|------------------------------------|-----------------------------|-------------------------------|-----------------------------------|---------------------------------------------------|
| 29  | K         | COMPARATIVE EXAMPLE | <u>1.00</u>                        | UNDONE                      | 1200                          | 60                                | 20                                                |
| 30  | K         | COMPARATIVE EXAMPLE | <u>0.70</u>                        | <u>1150° C. x 5 h</u>       | 1200                          | 60                                | 20                                                |
| 31  | K         | COMPARATIVE EXAMPLE | <u>0.70</u>                        | <u>1200° C. x 15 m</u>      | 1200                          | 60                                | 20                                                |
| 32  | K         | COMPARATIVE EXAMPLE | 0.45                               | 1250° C. x 4 h              | <u>1350</u>                   | 60                                | 20                                                |
| 33  | K         | COMPARATIVE EXAMPLE | 0.40                               | 1250° C. x 4 h              | <u>1050</u>                   | <u>0</u>                          | 68                                                |
| 34  | K         | COMPARATIVE EXAMPLE | 0.30                               | 1250° C. x 4 h              | 1200                          | 60                                | <u>7</u>                                          |
| 35  | K         | COMPARATIVE EXAMPLE | <u>0.75</u>                        | 1250° C. x 4 h              | 1200                          | 60                                | 20                                                |
| 36  | K         | COMPARATIVE EXAMPLE | <u>0.75</u>                        | 1250° C. x 4 h              | 1200                          | 60                                | 20                                                |
| 37  | K         | COMPARATIVE EXAMPLE | 0.00                               | 1250° C. x 4 h              | 1200                          | 60                                | 20                                                |
| 38  | L         | EXAMPLE             | 0.30                               | 1250° C. x 4 h              | 1200                          | 60                                | 20                                                |
| 39  | M         | EXAMPLE             | 0.35                               | 1250° C. x 4 h              | 1200                          | 60                                | 20                                                |
| 40  | N         | EXAMPLE             | 0.25                               | 1250° C. x 4 h              | 1200                          | 60                                | 20                                                |

      : VALUE WITHOUT THE RANGE OF THE PRESENT INVENTION

TABLE 3-2

| No. | STEEL No. | ROLLING FINISHING TEMPERATURE (° C.) | COOLING RATE AT A TEMPERA-TURE OF 800 TO 500° C. (° C./min) | SOLUTION HEAT TREATMENT | EAR CRACK (mm) | PROOF STRESS (MPa) | V <sub>C</sub> 100 vE-40° C. (J/cm <sup>2</sup> ) | (mV vs Saturated Ag/AgCl) |     |
|-----|-----------|--------------------------------------|-------------------------------------------------------------|-------------------------|----------------|--------------------|---------------------------------------------------|---------------------------|-----|
| 24  | K         | EXAMPLE                              | 900                                                         | 250                     | UNDONE         | 0                  | 740                                               | 183                       | 700 |
| 25  | K         | EXAMPLE                              | 900                                                         | 250                     | UNDONE         | 0                  | 745                                               | 182                       | 695 |
| 26  | K         | EXAMPLE                              | 860                                                         | 250                     | UNDONE         | 0                  | 751                                               | 167                       | 695 |
| 27  | K         | EXAMPLE                              | 970                                                         | 250                     | UNDONE         | 0                  | 723                                               | 197                       | 700 |
| 28  | K         | EXAMPLE                              | 900                                                         | 500                     | UNDONE         | 0                  | 741                                               | 193                       | 715 |
| 29  | K         | COMPARATIVE EXAMPLE                  | 900                                                         | 250                     | UNDONE         | 0                  | 743                                               | <u>53</u>                 | 645 |
| 30  | K         | COMPARATIVE EXAMPLE                  | 900                                                         | 250                     | UNDONE         | 0                  | 741                                               | <u>60</u>                 | 655 |
| 31  | K         | COMPARATIVE EXAMPLE                  | 900                                                         | 250                     | UNDONE         | 0                  | 740                                               | <u>63</u>                 | 655 |
| 32  | K         | COMPARATIVE EXAMPLE                  | 900                                                         | 250                     | UNDONE         | 70                 | 720                                               | <u>95</u>                 | 605 |
| 33  | K         | COMPARATIVE EXAMPLE                  | 900                                                         | 250                     | UNDONE         | 0                  | 755                                               | <u>66</u>                 | 705 |
| 34  | K         | COMPARATIVE EXAMPLE                  | 900                                                         | 250                     | UNDONE         | 0                  | <u>545</u>                                        | 270                       | 715 |
| 35  | K         | COMPARATIVE EXAMPLE                  | <u>800</u>                                                  | 250                     | UNDONE         | 0                  | 752                                               | <u>52</u>                 | 585 |
| 36  | K         | COMPARATIVE EXAMPLE                  | 900                                                         | <u>75</u>               | UNDONE         | 0                  | 743                                               | <u>47</u>                 | 570 |
| 37  | K         | COMPARATIVE EXAMPLE                  | 900                                                         | 250                     | <u>DONE</u>    | 0                  | <u>358</u>                                        | 304                       | 815 |
| 38  | L         | EXAMPLE                              | 900                                                         | 250                     | UNDONE         | 0                  | 652                                               | 197                       | 735 |
| 39  | M         | EXAMPLE                              | 900                                                         | 250                     | UNDONE         | 0                  | 700                                               | 191                       | 720 |
| 40  | N         | EXAMPLE                              | 900                                                         | 250                     | UNDONE         | 0                  | 758                                               | 183                       | 645 |

      : VALUE WITHOUT THE RANGE OF THE PRESENT INVENTION

TABLE 4-1

| No. | STEEL No. |                     | INTERMETALLIC COMPOUND CONTENT (%) | HOMOGENIZING HEAT TREATMENT | RE-HEATING TEMPERATURE (° C.) | REDUCTION AT 1050° C. OR MORE (%) | REDUCTION AT A TEMPERATURE OF 1050 TO 850° C. (%) |
|-----|-----------|---------------------|------------------------------------|-----------------------------|-------------------------------|-----------------------------------|---------------------------------------------------|
| 41  | a         | COMPARATIVE EXAMPLE | 0.40                               | 1250° C. x 4 h              | 1200                          | 60                                | 20                                                |
| 42  | b         | COMPARATIVE EXAMPLE | 0.35                               | 1250° C. x 4 h              | 1200                          | 60                                | 20                                                |

TABLE 4-1-continued

| No. | STEEL No. |                        | INTERMETALLIC<br>COMPOUND<br>CONTENT (%) | HOMOGENIZING<br>HEAT<br>TREATMENT | RE-HEATING<br>TEMPERATURE<br>(° C.) | REDUCTION<br>AT 1050° C.<br>OR MORE (%) | REDUCTION AT A<br>TEMPERATURE OF<br>1050 TO 850° C. (%) |
|-----|-----------|------------------------|------------------------------------------|-----------------------------------|-------------------------------------|-----------------------------------------|---------------------------------------------------------|
| 43  | c         | COMPARATIVE<br>EXAMPLE | 0.45                                     | 1250° C. × 4 h                    | 1200                                | 60                                      | 20                                                      |
| 44  | d         | COMPARATIVE<br>EXAMPLE | 0.05                                     | 1250° C. × 4 h                    | 1200                                | 60                                      | 20                                                      |
| 45  | e         | COMPARATIVE<br>EXAMPLE | 0.20                                     | 1250° C. × 4 h                    | 1200                                | 60                                      | 20                                                      |
| 46  | f         | COMPARATIVE<br>EXAMPLE | 0.50                                     | 1250° C. × 4 h                    | 1200                                | 60                                      | 20                                                      |
| 47  | g         | COMPARATIVE<br>EXAMPLE | 0.13                                     | 1250° C. × 4 h                    | 1200                                | 60                                      | 20                                                      |
| 48  | h         | COMPARATIVE<br>EXAMPLE | <u>0.95</u>                              | 1250° C. × 4 h                    | 1200                                | 60                                      | 20                                                      |
| 49  | i         | COMPARATIVE<br>EXAMPLE | 0.40                                     | 1250° C. × 4 h                    | 1200                                | 60                                      | 20                                                      |
| 50  | j         | COMPARATIVE<br>EXAMPLE | 0.30                                     | 1250° C. × 4 h                    | 1200                                | 60                                      | 20                                                      |
| 51  | k         | COMPARATIVE<br>EXAMPLE | 0.15                                     | 1250° C. × 4 h                    | 1200                                | 60                                      | 20                                                      |
| 52  | l         | COMPARATIVE<br>EXAMPLE | <u>0.90</u>                              | 1250° C. × 4 h                    | 1200                                | 60                                      | 20                                                      |
| 53  | m         | COMPARATIVE<br>EXAMPLE | 0.00                                     | 1250° C. × 4 h                    | 1200                                | 60                                      | 20                                                      |
| 54  | n         | COMPARATIVE<br>EXAMPLE | 0.25                                     | 1250° C. × 4 h                    | 1200                                | 60                                      | 20                                                      |
| 55  | o         | COMPARATIVE<br>EXAMPLE | 0.30                                     | 1250° C. × 4 h                    | 1200                                | 60                                      | 20                                                      |
| 56  | p         | COMPARATIVE<br>EXAMPLE | 0.10                                     | 1250° C. × 4 h                    | 1200                                | 60                                      | 20                                                      |
| 57  | q         | COMPARATIVE<br>EXAMPLE | 0.20                                     | 1250° C. × 4 h                    | 1200                                | 60                                      | 20                                                      |
| 58  | r         | COMPARATIVE<br>EXAMPLE | 0.15                                     | 1250° C. × 4 h                    | 1200                                | 60                                      | 20                                                      |
| 59  | s         | COMPARATIVE<br>EXAMPLE | 0.30                                     | 1250° C. × 4 h                    | 1200                                | 60                                      | 20                                                      |
| 60  | t         | COMPARATIVE<br>EXAMPLE | 0.30                                     | 1250° C. × 4 h                    | 1200                                | 60                                      | 20                                                      |
| 61  | u         | COMPARATIVE<br>EXAMPLE | 0.30                                     | 1250° C. × 4 h                    | 1200                                | 60                                      | 20                                                      |
| 62  | v         | COMPARATIVE<br>EXAMPLE | 0.15                                     | 1250° C. × 4 h                    | 1200                                | 60                                      | 20                                                      |
| 63  | w         | COMPARATIVE<br>EXAMPLE | 0.10                                     | 1250° C. × 4 h                    | 1200                                | 60                                      | 20                                                      |

  : VALUE WITHOUT THE RANGE OF THE PRESENT INVENTION

TABLE 4-2

| No. | STEEL No. | ROLLING<br>FINISHING<br>TEMPERATURE<br>(° C.) | COOLING<br>RATE AT A<br>TEMPERA-<br>TURE OF 800<br>TO 500° C.<br>(° C./min) | SOLUTION<br>HEAT<br>TREATMENT | EAR<br>CRACK<br>(mm) | PROOF<br>STRESS<br>(MPa) | vE-40° C.<br>(J/cm <sup>2</sup> ) | Vc' 100<br>(mV vs<br>Saturated<br>Ag/AgCl) |            |
|-----|-----------|-----------------------------------------------|-----------------------------------------------------------------------------|-------------------------------|----------------------|--------------------------|-----------------------------------|--------------------------------------------|------------|
| 41  | a         | COMPARATIVE<br>EXAMPLE                        | 900                                                                         | 250                           | UNDONE               | 5                        | 695                               | 199                                        | <u>455</u> |
| 42  | b         | COMPARATIVE<br>EXAMPLE                        | 900                                                                         | 250                           | UNDONE               | 10                       | 726                               | <u>65</u>                                  | 730        |
| 43  | c         | COMPARATIVE<br>EXAMPLE                        | 900                                                                         | 250                           | UNDONE               | 8                        | 705                               | <u>77</u>                                  | <u>490</u> |
| 44  | d         | COMPARATIVE<br>EXAMPLE                        | 900                                                                         | 250                           | UNDONE               | 50                       | 728                               | <u>75</u>                                  | 550        |
| 45  | e         | COMPARATIVE<br>EXAMPLE                        | 900                                                                         | 250                           | UNDONE               | 45                       | 700                               | <u>53</u>                                  | <u>435</u> |
| 46  | f         | COMPARATIVE<br>EXAMPLE                        | 900                                                                         | 250                           | UNDONE               | 0                        | 752                               | <u>71</u>                                  | 520        |
| 47  | g         | COMPARATIVE<br>EXAMPLE                        | 900                                                                         | 250                           | UNDONE               | 6                        | 644                               | 310                                        | <u>405</u> |
| 48  | h         | COMPARATIVE<br>EXAMPLE                        | 900                                                                         | 250                           | UNDONE               | 9                        | 644                               | <u>30</u>                                  | 765        |
| 49  | i         | COMPARATIVE<br>EXAMPLE                        | 900                                                                         | 250                           | UNDONE               | 0                        | 621                               | 195                                        | <u>470</u> |
| 50  | j         | COMPARATIVE<br>EXAMPLE                        | 900                                                                         | 250                           | UNDONE               | 12                       | 718                               | <u>35</u>                                  | 510        |

TABLE 4-2-continued

| No. | STEEL No. | COMPARATIVE EXAMPLE | ROLLING FINISHING TEMPERATURE (° C.) | COOLING RATE AT A TEMPERA-TURE OF 800 TO 500° C. (° C./min) | SOLUTION HEAT TREATMENT | EAR CRACK (mm) | PROOF STRESS (MPa) | vE-40° C. (J/cm²) | Vc' 100 (mV vs Saturated Ag/AgCl) |
|-----|-----------|---------------------|--------------------------------------|-------------------------------------------------------------|-------------------------|----------------|--------------------|-------------------|-----------------------------------|
|     |           |                     |                                      |                                                             |                         |                |                    |                   |                                   |
| 51  | k         | COMPARATIVE EXAMPLE | 900                                  | 250                                                         | UNDONE                  | 0              | 685                | 222               | <u>205</u>                        |
| 52  | l         | COMPARATIVE EXAMPLE | 900                                  | 250                                                         | UNDONE                  | 33             | 740                | <u>20</u>         | 750                               |
| 53  | m         | COMPARATIVE EXAMPLE | 900                                  | 250                                                         | UNDONE                  | 0              | 715                | 215               | 660                               |
| 54  | n         | COMPARATIVE EXAMPLE | 900                                  | 250                                                         | UNDONE                  | 0              | 713                | <u>30</u>         | 655                               |
| 55  | o         | COMPARATIVE EXAMPLE | 900                                  | 250                                                         | UNDONE                  | 42             | 703                | 150               | <u>445</u>                        |
| 56  | p         | COMPARATIVE EXAMPLE | 900                                  | 250                                                         | UNDONE                  | 38             | 731                | 156               | <u>430</u>                        |
| 57  | q         | COMPARATIVE EXAMPLE | 900                                  | 250                                                         | UNDONE                  | 56             | 699                | 164               | <u>405</u>                        |
| 58  | r         | COMPARATIVE EXAMPLE | 900                                  | 250                                                         | UNDONE                  | 60             | 705                | 142               | 565                               |
| 59  | s         | COMPARATIVE EXAMPLE | 900                                  | 250                                                         | UNDONE                  | 0              | 713                | <u>61</u>         | 695                               |
| 60  | t         | COMPARATIVE EXAMPLE | 900                                  | 250                                                         | UNDONE                  | 0              | 666                | <u>52</u>         | 585                               |
| 61  | u         | COMPARATIVE EXAMPLE | 900                                  | 250                                                         | UNDONE                  | 0              | 720                | <u>30</u>         | 695                               |
| 62  | v         | COMPARATIVE EXAMPLE | 900                                  | 250                                                         | UNDONE                  | 0              | 735                | <u>70</u>         | 650                               |
| 63  | w         | COMPARATIVE EXAMPLE | 900                                  | 250                                                         | UNDONE                  | 0              | 696                | <u>21</u>         | 550                               |

      : VALUE WITHOUT THE RANGE OF THE PRESENT INVENTION

The steel plate produced under the above condition was cut into JIS. No. 4 tension test pieces and JIS. No. 4 V notch Charpy test pieces from a direction perpendicular to the direction of rolling processing. Using the resultant test pieces, 0.2% offset proof stress and impact strength at -40° C. were measured, and further the surface of the test piece was ground with a #600 grinder and then pitting electrical potential (Vc'100) was measured in a deaerated 10% NaCl aqueous solution held at 50° C. Moreover, test pieces for micro structure observation were cut out, and each of the resultant test pieces was planished and thereafter was subjected to 10% KOH electrolytic etching to reveal intermetallic compound therefrom so as to be observed by an optical microscope, thereby measuring the content. The content was measured by performing point counting in each of ten fields of view with 400 $\times$  magnification at a depth of each of  $\frac{1}{4}$ ,  $\frac{1}{2}$ , and  $\frac{3}{4}$  of thick, and then calculating all average values, and the resultant value was determined as the content of the intermetallic compound of the steel material. The obtained results are shown in Tables 2-4.

The hot-rolling processability was evaluated relatively by judging the generation of an ear crack during the product rolling. It was confirmed that the steel material corresponding to Example 4 to 6 (steel Nos. F to N) developed no ear cracks and exhibited excellent hot-rolling processability, with the exception of the case in which the reheating temperature was excessively high. On the other hand, it was confirmed that each of the steel materials corresponding to each Example other than Examples 4 to 6 developed ear cracks of approximately 5 to 10 mm per one side, so that the yield was decreased slightly. The lengths of ear cracks are shown in Tables 2 to 4.

As provided in the results shown in Tables 1 and 2-4, regarding the steel material which satisfies the steel composition which is within the scope of the present invention, the

intermetallic compound content, production condition, all of the corrosion resistance, the proof stress, and Charpy impact value satisfy the specified conditions.

As can be seen from the above examples, it is clarified that the steel material according to the exemplary embodiments of the present invention is an austenitic stainless steel material which excels in corrosion resistance, toughness, and strength.

The exemplary embodiments of the present invention provide an austenitic stainless steel suitable for the hull structures of ships, having excellent performance required for structural members of high-speed ships, such as sea water resistance, proof stress, and low-temperature toughness at a high level, and hence the contributions of the present invention to industry are significant.

The eighth exemplary embodiment of the present invention is described as follows

The content of C can be provided to be not more than 0.03%, in order to secure the corrosion resistance of the stainless steel. If the content of C exceeds 0.03%, then Cr carbide will be generated and corrosion resistance and toughness will deteriorate.

The content of Si is not less than 0.1% for deoxidation. However, if the content of Si exceeds 1.5%, then toughness will deteriorate. Therefore, the upper limit thereof is restricted to 1.5%. The content of Si preferably ranges from 0.2 to 1.0%.

The content of Mn is not less than 0.1% for deoxidation. However, if the content of Mn exceeds 3.0%, then corrosion resistance and toughness will deteriorate. Therefore, the upper limit thereof is restricted to 3.0%. The content of Mn preferably ranges from 0.2 to 1.5%.

The content of P is restricted to not more than 0.05% because P deteriorates hot-rolling processability and toughness. The content of P is preferably not more than 0.03%.

25

The content of S is restricted to not more than 0.003% because S deteriorates hot-rolling processability, toughness, and corrosion resistance. The content of S is preferably not more than 0.001%.

The content of Ni is not less than 15.0% because Ni stabilizes an austenitic phase, and improves resistance to various acids and toughness. On the other hand, Ni is an expensive metal, and hence the content of Ni is restricted to not more than 21.0% from the viewpoint of cost.

The content of Cr is not less than 22.0% for securing basic corrosion resistance. On the other hand, if the content of Cr exceeds 28.0%, then an intermetallic compound will likely be deposited to deteriorate toughness. For this reason, the content of Cr is restricted to not less than 22.0% and not more than 28.0%.

The content of Mo is not less than 1.5% in the present invention, because Mo is a very effective element which increases corrosion resistance of stainless steel additionally. On the other hand, Mo is a very expensive element and which accelerates the deposition of intermetallic compounds, as well as Cr, and hence the upper limit of the content of Mo is restricted to not more than 3.5%. The content of Mo preferably ranges from 2.0 to 3.0%.

N is an effective element which is intercrystallized into an austenitic phase to increase strength and corrosion resistance. For this reason, the content of N is not less than 0.15%. Although it is possible to make N be intercrystallized into the base material up to 0.4% in the steel material of the present invention, the upper limit of the content of N is determined as 0.35% in order to increase sensitivity to generation of bubbling during welding. The content of N is preferably not more than 0.30%.

Al is an important element for deoxidation of steel, and hence the content of Al is not less than 0.005% in order to reduce oxygen in steel. On the other hand, Al is an element having a comparatively high chemical affinity with N, and if the content of Al is excessive, then AlN is generated to deteriorate toughness of the stainless steel. Although the degree thereof depends on the content of N, if the content of Al exceeds 0.1%, then toughness will deteriorate significantly, and hence the upper limit of the content of Al is determined to be 0.1%.

O is an important element which constitutes an oxide which is a representative nonmetallic inclusion, and excessive addition of O deteriorates toughness, on the other hand if a coarse cluster-like oxide generates, then it causes surface cracking. For this reason, the upper limit of the content of O is determined as 0.007%. The content of O is preferably not more than 0.004%.

The PI value expressed by the above-mentioned formula (1): A pitting index is an index of corrosion resistance of stainless steel to a chloride environment, and it is necessary to set the PI value to be not less than 35 at least, in order to acquire the corrosion resistance corresponding to the purpose. As a stainless steel of which the PI value exceeds 40, SUS836L etc., is exemplary, however, such a stainless steel contains Ni in an amount of not less than 24% and hence is very expensive. In the present invention, since the aim is to provide austenitic stainless steel which has corrosion resistance corresponding to cost, the upper limit of PI value is determined to be 40. Note, the value of W in formula (1) is set to 0 in the present invention which does not contain W.

The  $\delta_{cal}$  expressed by the above-mentioned formula (2) is an index indicating the quantity of the delta ferrite which appears in the solidified configuration of austenitic stainless steel, and the  $\delta_{cal}$  is in general controlled to be approximately 0 to 7% in order to reduce solidification crack sensitivity or to

26

make the configuration fine. However, as in the stainless steel of the present invention having a high content of Cr, delta ferrite in the solidified configuration changes into an intermetallic compound during the hot-rolling production process and it remains in the steel material as a by-product, thereby deteriorating toughness. For this reason, the upper limit of the  $\delta_{cal}$  is restricted to +4 so that delta ferrite will decrease. If the  $\delta_{cal}$  exceeds this value, then it becomes impossible to acquire high toughness even if elaborating a plan in the hot-rolling production process. On the other hand, if the  $\delta_{cal}$  is shifted to a smaller (minus) side, then it means that the delta ferrite content becomes substantially 0%, and as a result the above effect will be saturated, in addition, the content of Ni becomes excessive, and hence the lower limit of the  $\delta_{cal}$  is determined to be -6 from the viewpoint of cost. The  $\delta_{cal}$  value preferably ranges from -3 to +3. Note, the value of W or the value of Cu in formula (2) is set to 0 in the exemplary embodiment of the present invention which does not contain W or Cu.

The content of intermetallic compounds contained in the steel material is an important factor which determines the toughness of the austenitic stainless steel material in the present invention. An intermetallic compound is a compound which contains Cr, Mo, or W as a main ingredient and is called  $\sigma$  phase and  $\chi$  phase. The content of this compound can be measured by subjecting a micro configuration to an alkaline electrolytic etching and then observing the resultant micro configuration through an optical microscope of approximately 400 $\times$  power. The inventors of the present invention have found that if this content as an average value of a stainless steel cross sectional observation exceeds 0.5%, then the Charpy absorbed energy of the steel material becomes less than 100 J/cm<sup>2</sup>, and as a result, they determined the upper limit of the content to be 0.5%.

The ninth exemplary embodiment of the present invention is described as follows

Cu is an element which increases the corrosion resistance of stainless steel additionally against an acid, and the content of Cu may be not less than 0.1% for this purpose. Even if the content Cu exceeds 2.0%, the effect corresponding to cost will be saturated, and hence the upper limit of the content of Cu is set to be 2.0%.

Ti is an element which forms an oxide, a nitride, and sulfide with a very small amount thereof, thereby refining the crystal grain of the steel, and hence Ti is an element which may be positively utilized in the steel of the present invention. In order to reduce the intermetallic compound content in the steel material, it is effective to restrict the upper limit of the  $\delta_{cal}$  value and to perform homogenizing heat treatment of the semi-finished products. Among these, in the latter method, although a heat treatment is performed for several hours at a high temperature of approximately 1250°C., if Ti of a proper amount is contained, then the growth of the crystal grain at such a high temperature can be suppressed. For this purpose, Ti in an amount of not less than 0.003% needs to be contained. On the other hand, Ti is an element which has a very high nitride producing ability, and if the content of Ti exceeds 0.03% in the steel of the present invention which contains N, then coarse TiN will deteriorate the toughness of the steel. For this reason, the content of Ti is determined to be within the range of 0.003 to 0.03%. The content of Ti preferably ranges from 0.005 to 0.02%.

Nb forms carbide to fix C, so that generation of Cr carbide is suppressed, thereby increasing corrosion resistance and toughness. Moreover, Nb forms nitride to suppress growth of crystal grain, thereby converting the steel material into fine particles to increase strength. In order to improve corrosion resistance and to increase strength, not less than 0.02% of Nb

can be added. However, if more than 0.2% of Nb is added, then a large amount of carbo-nitride of Nb will be deposited during the hot-rolling processing to deteriorate hot-rolling recrystallization, thereby maintaining a coarse configuration in the steel material as a product, and hence the upper limit of the content of Nb is determined to be 2%. The content of Nb preferably ranges from 0.05 to 0.15%.

V is an element which generates a carbo-nitride as well as Nb, and can be added in order to secure corrosion resistance and toughness. Although not less than 0.05% of V should be contained for this purpose, if more than 0.5% of V is contained, then coarse V series carbo-nitride will be generated, so that toughness will deteriorate conversely. Therefore, the upper limit of the content of V is restricted to 0.5%. Preferably, the content of V can have a range from 0.1 to 0.3%.

W is an element which raises the corrosion resistance of stainless steel additionally as well as Mo, and 0.3 to 3.0% of W can be contained in the stainless steel of the exemplary embodiment of the present invention for this exemplary purpose.

Furthermore, each of B, Ca, Mg, and REM(s) is an element which improves the hot-rolling processability, and one or more of these is added for this purpose. If any of these is added in excess, then it deteriorates the hot-rolling processability, and hence the upper limit and the lower limit of content thereof are determined as follows. The content of B ranges from 0.0003 to 0.0060%, each of the content of Ca and Mg ranges from 0.0005 to 0.0050%, and the content of REM ranges from 0.005 to 0.10%. Here, REM is defined to be the total of the content of lanthanide series rare-earth elements such as La, Ce, etc.

The tenth exemplary embodiment of the present invention is described as follows

In order to raise the toughness of steel materials in the present invention, the amount of intermetallic compound which is contained in the steel material is restricted to be not more than 0.5%. To achieve this, a chemical composition formula known as  $\delta$  cal, which forecasts delta ferrite amount contained in a solidification structure configuration, and homogenizing heat treatment which is performed on a semi-

finished product specified in this exemplary embodiment are exemplary. When there is no solidifying segregation in the target steel material of the present invention, the temperature at which an intermetallic compound is generated is approximately not higher than 1000° C. However, reduction of the content of an intermetallic compound in the semi-finished product accompanied by component segregation by solidification necessitates a production step for diffusing segregation so as to be homogenized. Although each of the temperature and the time for performing homogenizing heat treatment changes slightly, depending on chemical composition such as solidifying rate, cross-sectional area of a cast steel, degree of hot-rolling processing upon being shaped into a semi-finished product,  $\delta$  cal, etc., each of the temperature and the time for performing homogenizing heat treatment is limited by diffusion of Cr, Mo, Ni, etc., and hence it necessitates a temperature of not lower than 1200° C. On the other hand, if the temperature exceeds 1300° C., then oxidized scales may be generated extraordinarily.

Moreover, although it is preferred that the time be as long as possible, at least 1 hour is needed. Moreover, this purpose can also be attained by performing soaking at 1200° C. for not less than 1 hour in heating of the semi-finished product for rolling the product. Because of the above reason, homogenizing heat treatment of not less than 1 hour at 1200-1300° C. is specified. In view of effect and economical efficiency, the soaking time preferably ranges from 2 to 20 hours.

## EXAMPLE 2

The chemical composition of a sample steel is shown in Table 5 herein. The content of inevitable impurity elements other than the components indicated in Table 5 is the same grade as in standard stainless steel. Moreover, the portion which shows no content of the components shown in Table 5 indicates the same grade as in impurities. In addition, REM in Table 5 means lanthanide series rare-earth elements, and the content thereof indicates the total content of each of those elements.

Each of these steels was melted in a 50 kg vacuum induction furnace of a laboratory, and each of them was cast into a flat steel ingot having a thickness of approximately 100 mm.

TABLE 5-1

| STEEL No. | KIND                      | CONTENT (mass %) |      |      |       |        |       |       |      |      |       |       |
|-----------|---------------------------|------------------|------|------|-------|--------|-------|-------|------|------|-------|-------|
|           |                           | C                | Si   | Mn   | P     | S      | Ni    | Cr    | Mo   | Cu   | Nb    | Ti    |
| 0         | EXAMPLE 7                 | 0.019            | 0.51 | 0.45 | 0.023 | 0.0005 | 18.03 | 25.01 | 2.48 |      |       |       |
| 1         | EXAMPLE 8                 | 0.021            | 0.49 | 0.48 | 0.020 | 0.0007 | 17.91 | 25.24 | 2.50 | 0.15 |       |       |
| 2         | EXAMPLE 8                 | 0.018            | 0.52 | 0.52 | 0.014 | 0.0012 | 17.98 | 25.02 | 2.46 |      |       | 0.008 |
| 3         | EXAMPLE 9                 | 0.022            | 0.49 | 0.52 | 0.022 | 0.0008 | 18.43 | 24.88 | 2.46 | 0.29 | 0.096 |       |
| 4         | EXAMPLE 9                 | 0.021            | 0.48 | 0.52 | 0.022 | 0.0007 | 17.38 | 25.36 | 2.53 | 0.30 | 0.034 | 0.006 |
| 5         | EXAMPLE 9                 | 0.022            | 0.46 | 0.52 | 0.021 | 0.0008 | 20.21 | 24.96 | 2.46 | 0.31 | 0.103 | 0.015 |
| 6         | EXAMPLE 9                 | 0.022            | 0.48 | 0.49 | 0.022 | 0.0003 | 19.23 | 24.32 | 3.33 | 0.28 |       |       |
| 7         | EXAMPLE 9                 | 0.021            | 0.47 | 0.52 | 0.022 | 0.0007 | 18.33 | 24.66 | 2.48 | 0.32 |       | 0.005 |
| 8         | EXAMPLE 9                 | 0.019            | 0.45 | 0.53 | 0.023 | 0.0008 | 18.23 | 24.65 | 2.46 | 0.32 |       | 0.003 |
| 9         | EXAMPLE 9                 | 0.021            | 0.48 | 0.51 | 0.023 | 0.0008 | 18.52 | 24.03 | 2.46 | 0.32 |       | 0.006 |
| 10        | EXAMPLE 9                 | 0.019            | 0.49 | 0.49 | 0.022 | 0.0004 | 20.42 | 27.31 | 1.68 | 0.31 | 0.042 | 0.006 |
| 11        | EXAMPLE 9                 | 0.024            | 0.49 | 0.49 | 0.021 | 0.0003 | 19.53 | 25.61 | 2.11 | 1.82 |       | 0.012 |
| 12        | EXAMPLE 9                 | 0.019            | 0.49 | 0.85 | 0.019 | 0.0013 | 18.89 | 25.29 | 2.52 | 0.32 | 0.076 | 0.004 |
| 13        | EXAMPLE 9                 | 0.021            | 0.50 | 0.84 | 0.019 | 0.0005 | 16.77 | 24.66 | 2.10 | 0.85 |       | 0.006 |
| 14        | EXAMPLE 9                 | 0.021            | 0.26 | 1.85 | 0.022 | 0.0009 | 19.53 | 24.33 | 3.45 | 0.31 | 0.152 | 0.022 |
| 15        | EXAMPLE 9                 | 0.018            | 0.56 | 0.53 | 0.021 | 0.0006 | 16.95 | 22.21 | 3.39 | 1.66 |       | 0.007 |
| 21        | COMPARATIVE               | 0.021            | 0.48 | 0.53 | 0.023 | 0.0008 | 18.23 | 24.89 | 2.46 | 0.32 |       | 0.046 |
|           | STEEL EXAMPLE             |                  |      |      |       |        |       |       |      |      |       |       |
| 22        | COMPARATIVE STEEL EXAMPLE | 0.022            | 0.47 | 0.54 | 0.024 | 0.0007 | 18.33 | 25.00 | 2.45 | 0.35 | 0.284 |       |

TABLE 5-1-continued

| STEEL No. | KIND                      | CONTENT (mass %) |      |      |       |        |              |       |      |      |    |    |
|-----------|---------------------------|------------------|------|------|-------|--------|--------------|-------|------|------|----|----|
|           |                           | C                | Si   | Mn   | P     | S      | Ni           | Cr    | Mo   | Cu   | Nb | Ti |
| 23        | COMPARATIVE STEEL EXAMPLE | 0.023            | 0.46 | 0.55 | 0.023 | 0.0008 | 18.25        | 24.98 | 2.48 | 0.32 |    |    |
| 24        | COMPARATIVE STEEL EXAMPLE | 0.024            | 0.45 | 0.52 | 0.024 | 0.0006 | 18.22        | 24.94 | 2.47 | 0.31 |    |    |
| 25        | COMPARATIVE STEEL EXAMPLE | 0.022            | 0.47 | 0.53 | 0.025 | 0.0008 | 18.21        | 24.96 | 2.46 | 0.33 |    |    |
| 26        | COMPARATIVE STEEL EXAMPLE | 0.021            | 0.48 | 0.51 | 0.024 | 0.0007 | 17.01        | 25.11 | 2.88 | 0.31 |    |    |
| 27        | COMPARATIVE STEEL EXAMPLE | 0.022            | 0.49 | 0.52 | 0.023 | 0.0008 | <u>21.40</u> | 24.95 | 2.47 | 0.33 |    |    |

\_\_\_\_: VALUE WITHOUT THE RANGE OF THE PRESENT INVENTION

TABLE 5-2

| STEEL No. | KIND                      | CONTENT (mass %) |              |       |        |        |        |       |               |       |             |      |
|-----------|---------------------------|------------------|--------------|-------|--------|--------|--------|-------|---------------|-------|-------------|------|
|           |                           | V                | W            | Al    | B      | Ca     | Mg     | REM   | O             | N     | δ cal       | PI   |
| 0         | EXAMPLE 7                 |                  |              | 0.023 |        |        |        |       | 0.0027        | 0.275 | -1.1        | 37.6 |
| 1         | EXAMPLE 8                 |                  |              | 0.020 |        |        |        |       | 0.0046        | 0.235 | 1.7         | 37.3 |
| 2         | EXAMPLE 8                 |                  |              | 0.018 |        |        |        |       | 0.0041        | 0.266 | -0.5        | 37.4 |
| 3         | EXAMPLE 9                 | 0.06             |              | 0.032 |        | 0.0023 |        |       | 0.0018        | 0.240 | -1.3        | 36.8 |
| 4         | EXAMPLE 9                 |                  |              | 0.026 |        | 0.0022 |        |       | 0.0023        | 0.238 | 3.2         | 37.5 |
| 5         | EXAMPLE 9                 |                  |              | 0.028 |        | 0.0025 |        |       | 0.0025        | 0.242 | -5.8        | 37.0 |
| 6         | EXAMPLE 9                 | 0.15             |              | 0.034 | 0.0035 |        |        |       | 0.0019        | 0.257 | -3.3        | 39.4 |
| 7         | EXAMPLE 9                 |                  | 0.35         | 0.022 |        | 0.0025 |        |       | 0.0026        | 0.235 | -0.8        | 37.2 |
| 8         | EXAMPLE 9                 |                  | 1.05         | 0.023 |        | 0.0008 | 0.0033 |       | 0.0035        | 0.247 | -0.1        | 38.5 |
| 9         | EXAMPLE 9                 |                  | 2.10         | 0.024 |        | 0.0024 |        |       | 0.0029        | 0.241 | -0.9        | 39.5 |
| 10        | EXAMPLE 9                 |                  |              | 0.011 | 0.0023 | 0.0023 |        |       | 0.0036        | 0.245 | -1.6        | 36.8 |
| 11        | EXAMPLE 9                 | 0.28             |              | 0.023 |        | 0.0020 |        |       | 0.0025        | 0.173 | -0.7        | 35.3 |
| 12        | EXAMPLE 9                 |                  |              | 0.020 |        | 0.0008 |        | 0.050 | 0.0040        | 0.235 | -0.9        | 37.4 |
| 13        | EXAMPLE 9                 | 0.07             |              | 0.018 |        | 0.0042 |        |       | 0.0020        | 0.315 | -3.1        | 36.6 |
| 14        | EXAMPLE 9                 |                  |              | 0.020 |        | 0.0019 | 0.0008 |       | 0.0032        | 0.184 | -1.1        | 38.7 |
| 15        | EXAMPLE 9                 | 0.12             |              | 0.024 |        | 0.0030 |        |       | 0.0032        | 0.188 | -0.2        | 36.4 |
| 21        | COMPARATIVE STEEL EXAMPLE |                  |              | 0.026 |        | 0.0025 |        |       | 0.0032        | 0.241 | -0.7        | 36.9 |
| 22        | COMPARATIVE STEEL EXAMPLE |                  |              | 0.026 |        | 0.0026 |        |       | 0.0033        | 0.242 | -0.9        | 37.0 |
| 23        | COMPARATIVE STEEL EXAMPLE | <u>0.88</u>      |              | 0.024 |        | 0.0025 |        |       | 0.0031        | 0.239 | -0.6        | 37.0 |
| 24        | COMPARATIVE STEEL EXAMPLE |                  | <u>0.140</u> |       |        | 0.0024 |        |       | 0.0032        | 0.240 | -0.8        | 36.9 |
| 25        | COMPARATIVE STEEL EXAMPLE |                  | <u>0.002</u> |       |        | 0.0036 |        |       | <u>0.0081</u> | 0.242 | -0.6        | 37.0 |
| 26        | COMPARATIVE STEEL EXAMPLE |                  | 0.023        |       |        | 0.0022 |        |       | 0.0029        | 0.237 | <u>4.5</u>  | 38.4 |
| 27        | COMPARATIVE STEEL EXAMPLE |                  | 0.026        |       |        | 0.0023 |        |       | 0.0030        | 0.240 | <u>-8.8</u> | 36.9 |

\_\_\_\_: VALUE WITHOUT THE RANGE OF THE PRESENT INVENTION

The sample steel was subjected to cogging, homogenizing heat treatment, and product rolling. In the cogging, the sample steel was soaked at 1180°C. for two hours, and thereafter the sample steel was rolled to 65 mm thickness. Then the resultant semi-finished products were subjected to homogenizing heat treatment at a temperature ranging from 1220 to 1280°C. Some of the semi-finished products were not subjected to the homogenizing heat treatment. Each piece of steel was ground to 60 mm to obtain the material for use in

product rolling. In the product rolling, the sample was soaked at 1220°C. for 1 to 2 hours, and thereafter was rolled under the condition of a finishing temperature of 850 to 950°C. to obtain a steel sheet having a thickness of 12 mm. It should be noted that the steel material immediately after being hot-rolled which was in a temperature state of not less than 800°C. was cooled to a temperature of not higher than 300°C. by performing spray cooling. The final solution heat treatment was performed under a condition of cooling with water after

performing soaking at 1100° C. for 20 min. Moreover, some steel sheets were not subjected to the solution heat treatment.

The steel plate produced under the above condition was cut into JIS. No. 4 tension test pieces and JIS. No. 4 V notch Charpy test pieces from a direction perpendicular to the direction of rolling processing. Using the resultant test pieces, 0.2% offset proof stress and impact strength at -40° C. were measured. Moreover, test pieces for micro configuration observation were cut out, and each of the resultant test pieces was planished and thereafter was subjected to 10% KOH

electrolytic etching to reveal the intermetallic compound therefrom so as to be observed by an optical microscope, thereby measuring the content. The content was measured by performing point counting in each of ten fields of view with 400 $\times$  magnification at a depth of each of  $\frac{1}{4}$ ,  $\frac{1}{2}$ , and  $\frac{3}{4}$  of thickness, and then calculating all the average values, and the resultant value was determined as the content of the intermetallic compound of the steel material. The obtained results are shown in Table 6.

TABLE 6-1

| STEEL NO. | KIND                | INTERMETALLIC COMPOUND CONTENT (%) | HOMOGENIZING HEAT TREATMENT | ROLLING FINISHING TEMPERATURE (° C.) | SOLUTION HEAT TREATMENT | YS (MPa) | TS (MPa) | vE-40° C. (J/cm <sup>2</sup> ) | EAR CRACK (mm) |   |
|-----------|---------------------|------------------------------------|-----------------------------|--------------------------------------|-------------------------|----------|----------|--------------------------------|----------------|---|
| 0         | EXAMPLE             | 0.02                               | 1250° C. $\times$ 4 h       | 950                                  | DONE                    | 392      | 782      | 540                            | 6              |   |
| 0         | EXAMPLE             | 0.05                               | 1250° C. $\times$ 4 h       | 950                                  | DONE                    | 395      | 793      | 491                            | 9              |   |
| 0         | EXAMPLE             | 0.17                               | 1250° C. $\times$ 4 h       | 950                                  | UNDONE                  | 747      | 965      | 195                            | 6              |   |
| 0         | COMPARATIVE EXAMPLE | <u>0.75</u>                        | UNDONE                      | 850                                  | UNDONE                  | 892      | 1054     | 68                             | 12             |   |
| 1         | EXAMPLE             | 0.05                               | 1250° C. $\times$ 4 h       | 950                                  | DONE                    | 340      | 751      | 503                            | 6              |   |
| 1         | EXAMPLE             | 0.10                               | 1250° C. $\times$ 4 h       | 850                                  | DONE                    | 344      | 762      | 452                            | 8              |   |
| 1         | EXAMPLE             | 0.20                               | 1250° C. $\times$ 4 h       | 950                                  | UNDONE                  | 722      | 943      | 183                            | 5              |   |
| 1         | COMPARATIVE EXAMPLE | <u>1.2</u>                         | UNDONE                      | 850                                  | UNDONE                  | 841      | 1020     | 35                             | 10             |   |
| 2         | EXAMPLE             | 0.03                               | 1250° C. $\times$ 4 h       | 950                                  | DONE                    | 352      | 766      | 642                            | 5              |   |
| 2         | EXAMPLE             | 0.06                               | 1250° C. $\times$ 4 h       | 850                                  | DONE                    | 357      | 771      | 482                            | 7              |   |
| 2         | EXAMPLE             | 0.18                               | 1250° C. $\times$ 4 h       | 950                                  | UNDONE                  | 736      | 954      | 163                            | 5              |   |
| 2         | COMPARATIVE EXAMPLE | <u>0.8</u>                         | UNDONE                      | 850                                  | UNDONE                  | 882      | 1065     | 62                             | 10             |   |
| 3         | EXAMPLE             | 0.02                               | 1250° C. $\times$ 4 h       | 950                                  | DONE                    | 388      | 779      | 558                            | 0              |   |
| 3         | EXAMPLE             | 0.05                               | 1250° C. $\times$ 4 h       | 850                                  | DONE                    | 394      | 782      | 509                            | 0              |   |
| 3         | EXAMPLE             | 0.15                               | 1250° C. $\times$ 4 h       | 950                                  | UNDONE                  | 732      | 947      | 214                            | 0              |   |
| 3         | COMPARATIVE EXAMPLE | <u>0.7</u>                         | UNDONE                      | 850                                  | UNDONE                  | 865      | 1033     | 70                             | 0              |   |
| 3         | COMPARATIVE EXAMPLE | <u>0.55</u>                        | UNDONE                      | 900                                  | UNDONE                  | 812      |          | 982                            | 93             | 0 |
| 3         | EXAMPLE             | 0.42                               | UNDONE                      | 950                                  | UNDONE                  | 742      | 949      | 116                            | 0              |   |
| 4         | EXAMPLE             | 0.45                               | 1220° C. $\times$ 1 h       | 950                                  | UNDONE                  | 356      | 768      | 105                            | 0              |   |
| 4         | EXAMPLE             | 0.36                               | 1250° C. $\times$ 2 h       | 950                                  | UNDONE                  | 356      | 766      | 114                            | 0              |   |
| 4         | EXAMPLE             | 0.23                               | 1250° C. $\times$ 4 h       | 950                                  | UNDONE                  | 368      | 765      | 135                            | 0              |   |
| 4         | EXAMPLE             | 0.15                               | 1250° C. $\times$ 20 h      | 950                                  | UNDONE                  | 352      | 764      | 167                            | 0              |   |
| 4         | EXAMPLE             | 0.22                               | 1280° C. $\times$ 2 h       | 950                                  | UNDONE                  | 347      | 762      | 133                            | 0              |   |
| 5         | EXAMPLE             | 0.02                               | 1250° C. $\times$ 4 h       | 850                                  | DONE                    | 393      | 785      | 564                            | 0              |   |
| 5         | EXAMPLE             | 0.08                               | 1250° C. $\times$ 4 h       | 950                                  | UNDONE                  | 745      | 960      | 265                            | 0              |   |
| 6         | EXAMPLE             | 0.05                               | 1250° C. $\times$ 4 h       | 850                                  | DONE                    | 352      | 753      | 508                            | 0              |   |
| 6         | EXAMPLE             | 0.12                               | 1250° C. $\times$ 4 h       | 950                                  | UNDONE                  | 748      | 962      | 213                            | 0              |   |

  : VALUE WITHOUT THE RANGE OF THE PRESENT INVENTION

TABLE 6-2

| STEEL NO. | KIND    | INTERMETALLIC COMPOUND CONTENT (%) | HOMOGENIZING HEAT TREATMENT | ROLLING FINISHING TEMPERATURE (° C.) | SOLUTION HEAT TREATMENT | YS (MPa) | TS (MPa) | vE-40° C. (J/cm <sup>2</sup> ) | EAR CRACK (mm) |
|-----------|---------|------------------------------------|-----------------------------|--------------------------------------|-------------------------|----------|----------|--------------------------------|----------------|
| 7         | EXAMPLE | 0.04                               | 1250° C. $\times$ 4 h       | 850                                  | DONE                    | 348      | 753      | 526                            | 0              |
| 7         | EXAMPLE | 0.16                               | 1250° C. $\times$ 4 h       | 950                                  | UNDONE                  | 738      | 958      | 216                            | 0              |
| 8         | EXAMPLE | 0.06                               | 1250° C. $\times$ 4 h       | 850                                  | DONE                    | 362      | 772      | 492                            | 0              |
| 8         | EXAMPLE | 0.19                               | 1250° C. $\times$ 4 h       | 950                                  | UNDONE                  | 771      | 982      | 165                            | 0              |
| 9         | EXAMPLE | 0.08                               | 1250° C. $\times$ 4 h       | 850                                  | DONE                    | 388      | 795      | 421                            | 0              |
| 9         | EXAMPLE | 0.32                               | 1250° C. $\times$ 4 h       | 950                                  | UNDONE                  | 788      | 994      | 132                            | 0              |
| 10        | EXAMPLE | 0.03                               | 1250° C. $\times$ 4 h       | 850                                  | DONE                    | 352      | 765      | 502                            | 0              |
| 10        | EXAMPLE | 0.10                               | 1250° C. $\times$ 4 h       | 950                                  | UNDONE                  | 740      | 936      | 165                            | 0              |
| 11        | EXAMPLE | 0.05                               | 1250° C. $\times$ 4 h       | 850                                  | DONE                    | 324      | 711      | 513                            | 0              |
| 11        | EXAMPLE | 0.17                               | 1250° C. $\times$ 4 h       | 950                                  | UNDONE                  | 735      | 925      | 164                            | 0              |
| 12        | EXAMPLE | 0.05                               | 1250° C. $\times$ 4 h       | 850                                  | DONE                    | 362      | 776      | 501                            | 0              |
| 12        | EXAMPLE | 0.18                               | 1250° C. $\times$ 4 h       | 950                                  | UNDONE                  | 762      | 975      | 168                            | 0              |
| 13        | EXAMPLE | 0.05                               | 1250° C. $\times$ 4 h       | 850                                  | DONE                    | 375      | 783      | 523                            | 0              |
| 13        | EXAMPLE | 0.17                               | 1250° C. $\times$ 4 h       | 950                                  | UNDONE                  | 775      | 983      | 185                            | 0              |
| 14        | EXAMPLE | 0.11                               | 1250° C. $\times$ 4 h       | 850                                  | DONE                    | 342      | 741      | 481                            | 0              |
| 14        | EXAMPLE | 0.32                               | 1250° C. $\times$ 4 h       | 950                                  | UNDONE                  | 726      | 932      | 135                            | 0              |
| 15        | EXAMPLE | 0.09                               | 1250° C. $\times$ 4 h       | 850                                  | DONE                    | 348      | 738      | 475                            | 0              |
| 15        | EXAMPLE | 0.28                               | 1250° C. $\times$ 4 h       | 950                                  | UNDONE                  | 749      | 974      | 140                            | 0              |

TABLE 6-2-continued

| STEEL NO. | KIND                | INTERMETALLIC COMPOUND CONTENT (%) | HOMOGENIZING HEAT TREATMENT | ROLLING FINISHING TEMPERATURE (° C.) | SOLUTION HEAT TREATMENT | YS (MPa) | TS (MPa) | vE-40° C. (J/cm²) | EAR CRACK (mm) |
|-----------|---------------------|------------------------------------|-----------------------------|--------------------------------------|-------------------------|----------|----------|-------------------|----------------|
| 21        | COMPARATIVE EXAMPLE | 0.25                               | 1250° C. x 4 h              | 950                                  | UNDONE                  | 721      | 926      | 85                | 0              |
| 22        | COMPARATIVE EXAMPLE | 0.26                               | 1250° C. x 4 h              | 950                                  | UNDONE                  | 765      | 904      | 76                | 0              |
| 23        | COMPARATIVE EXAMPLE | 0.24                               | 1250° C. x 4 h              | 950                                  | UNDONE                  | 754      | 967      | 83                | 0              |
| 24        | COMPARATIVE EXAMPLE | 0.28                               | 1250° C. x 4 h              | 950                                  | UNDONE                  | 735      | 954      | 92                | 0              |
| 25        | COMPARATIVE EXAMPLE | 0.26                               | 1250° C. x 4 h              | 950                                  | UNDONE                  | 713      | 941      | 78                | 0              |
| 26        | COMPARATIVE EXAMPLE | <u>0.94</u>                        | 1250° C. x 4 h              | 950                                  | UNDONE                  | 735      | 943      | 45                | 0              |
| 27        | COMPARATIVE EXAMPLE | 0.06                               | 1250° C. x 4 h              | 950                                  | UNDONE                  | 742      | 926      | 198               | 0              |

—: VALUE WITHOUT THE RANGE OF THE PRESENT INVENTION

The hot-rolling processability was evaluated relatively by judging the generation of an ear crack during the product rolling. It was confirmed that the steel material corresponding to Example 9 (steel Nos. 3 to 15) developed no ear cracks and exhibited excellent hot-rolling processability. On the other hand, it was confirmed that each of the steel materials corresponding to each Example other than Examples 7 and 8 developed ear cracks of approximately 5 to 12 mm per one side, so that the yield was decreased slightly. The lengths of ear cracks are shown in Table 6. That is, although there is a slight problem in the hot-rolling processability of steel Nos. 0 to 2, in the thick steel which was produced to have the content of an intermetallic compound of not more than 0.5%, each Charpy impact value at -40° C. exceeds 100 J/cm<sup>2</sup>. As to the steel Nos. 3 to 15, which are those in which Al, B, Ca, Mg, REM are contained in order to improve hot-rolling processability, no ear cracks occurred. Moreover, in Examples of the present invention produced so as to have the content of an intermetallic compound of not more than 0.5%, each Charpy impact value at -40° C. exceeds 100 J/cm<sup>2</sup>.

Further, in each of the comparative examples of steel Nos. 21 to 27, the content of Ti is less than 0.03%, the content of Nb is more than 0.2%, the content of V is more than 0.5%, the content of Al is more than 0.1%, the content of O is more than 0.007%, the content of δFe is more than 3%, and the content of Ni is more than 21% (δFe<-6%), i.e. each is out of the scope of the present invention, and the comparative examples other than No. 27 have poor impact property. Although the comparative example of steel No. 27 excels in impact property, it has a high content of Ni and hence deviates from one of the objects of the present invention.

As is clear from the results shown in Tables 5 and 6, each of the steel materials which satisfy the steel composition and intermetallic compound content within the scope of the present invention has a PI value, which is an index of corrosion resistance, of not less than 35, and exhibits high strength and a Charpy impact value of not less than 100 J/cm<sup>2</sup>.

As can be seen from the above examples, it is clarified that the steel material of the exemplary embodiment of the present invention is an austenitic stainless steel material which excels in corrosion resistance, toughness, and hot-rolling processability.

The foregoing merely illustrates the principles of the invention. Various modifications and alterations to the described embodiments will be apparent to those skilled in the art in view of the teachings herein. It will thus be appre-

20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
791

Mo: about 1.5 to 3.5 mass %,  
N: about 0.15 to 0.35 mass %, and  
O: about 0.0005 to 0.007 mass %,  
wherein a PI value expressed by the following formula

ranges from about 35 to 40:  $PI=Cr+3.3(Mo+0.5W)+16N$ , and

a  $\delta$  cal value expressed by the following formula ranges from about -6 to +1:  $\delta cal=2.9(Cr+0.3Si+Mo+0.5W)-2.6(Ni+0.3Mn+0.25Cu+35C+20N)-18$ ,

a remnant of the steel material comprising Fe and inevitable impurities, reheating the treated material at a temperature of about 1100° C. to 1300° C.;

hot rolling the reheated material, wherein a temperature of at least about 850° C. is maintained, and the hot rolling includes a rough rolling stage, in which a total compaction is not less than about 50% at a temperature of not less than about 1050° C., and a final rolling stage, in which a total compaction is not less than about 10% at a temperature of about 1050° C. to 850° C., and after the rolling procedure is performed, cooling the rolled material from about 800° C. to 500° C. at an average cooling rate of at least about 150° C./min, without a solution treatment.

2. An austenitic stainless hot-rolled steel material having a superior corrosion resistance, a proof stress, and a low-temperature toughness, wherein a content of intermetallic compounds contained in the steel material is at most about 0.5 mass %, about 0.2% proof stress at a room temperature is at least about 550 MPa, a Charpy impact value measured using a V-notch test piece at about -40° C. is at least about 100 J/cm<sup>2</sup>, a pitting potential measured in a deaerated aqueous solution of about 10% NaCl at about 50° C. (Vc'100) is at least about 500 mV as compared to a saturated solution of Ag/AgCl, and wherein the austenitic stainless hot-rolled steel material is produced by a process comprising:

performing, at a temperature of 1200° C. to 1300° C. for at least about one hour, a homogenizing-heat treatment on a material which is at least one of a cast steel or a semi-finished product of the steel material which comprises:

C: about 0.001 to 0.03 mass %,

Si: about 0.1 to 1.5 mass %,

Mn: about 0.1 to 3.0 mass %,

P: about 0.005 to 0.05 mass %,

S: about 0.0001 to 0.003 mass %,

Ni: about 15.0 to 21.0 mass %,

Cr: about 22.0 to 28.0 mass %,

Mo: about 1.5 to 3.5 mass %,

N: about 0.15 to 0.35 mass %,

O: about 0.0005 to 0.007 mass %, and

at least one of:

W: about 0.3 to 3.0 mass %, or

Al: about 0.005 to 0.1 mass %,

wherein a PI value expressed by the following formula

ranges from about 35 to 40:  $PI=Cr+3.3(Mo+0.5W)+16N$ , and

a  $\delta$  cal value expressed by the following formula ranges from about -6 to +1:  $\delta cal=2.9(Cr+0.3Si+Mo+0.5W)-2.6(Ni+0.3Mn+0.25Cu+35C+20N)-18$ , and

a remnant of the steel material comprising Fe and inevitable impurities, reheating the treated material at a temperature of about 1100° C. to 1300° C.;

hot rolling the reheated material, wherein a temperature of at least about 850° C. is maintained, and the hot rolling includes a rough rolling stage, in which a total compac-

tion is not less than about 50% at a temperature of not less than about 1050° C., and a final rolling stage, in which a total compaction is not less than about 10% at a temperature of about 1050° C. to 850° C., and

after the rolling procedure is performed, cooling the rolled material from about 800° C. to 500° C. at an average cooling rate of at least about 150° C./min, without a solution treatment.

3. An austenitic stainless hot-rolled steel material having a superior corrosion resistance, a proof stress, and a low-temperature toughness, wherein a content of intermetallic compounds contained in the steel material is at most about 0.5 mass %, about 0.2% proof stress at a room temperature is at least about 550 MPa, a Charpy impact value measured using a V-notch test piece at about -40° C. is at least about 100 J/cm<sup>2</sup>, a pitting potential measured in a deaerated aqueous solution of about 10% NaCl at about 50° C. (Vc'100) is at least about 500 mV as compared to a saturated solution of Ag/AgCl, and wherein the austenitic stainless hot-rolled steel material is produced by a process comprising:

performing, at a temperature of 1200° C. to 1300° C. for at least about one hour, a homogenizing-heat treatment on a material which is at least one of a cast steel or a semi-finished product of the steel material which comprises:

C: about 0.001 to 0.03 mass %,

Si: about 0.1 to 1.5 mass %,

Mn: about 0.1 to 3.0 mass %,

P: about 0.005 to 0.05 mass %,

S: about 0.0001 to 0.003 mass %,

Ni: about 15.0 to 21.0 mass %;

Cr: about 22.0 to 28.0 mass %,

Mo: about 1.5 to 3.5 mass %,

N: about 0.15 to 0.35 mass %,

O: about 0.0005 to 0.007 mass %, and

at least one of:

W: about 0.3 to 3.0 mass %,

Al: about 0.005 to 0.1 mass %,

Cu: about 0.3 to 2.0 mass %, or

Sn: at most about 0.1 mass %,

wherein a PI value expressed by the following formula ranges from about 35 to 40:  $PI=Cr+3.3(Mo+0.5W)+16N$ , and

a  $\delta$  cal value expressed by the following formula ranges from about -6 to +1:  $\delta cal=2.9(Cr+0.3Si+Mo+0.5W)-2.6(Ni+0.3Mn+0.25Cu+35C+20N)-18$ , and

a remnant of the steel material comprising Fe and inevitable impurities, reheating the treated material at a temperature of about 1100° C. to 1300° C.;

hot rolling the reheated material, wherein a temperature of at least about 850° C. is maintained, and the hot rolling includes a rough rolling stage, in which a total compaction is not less than about 50% at a temperature of not less than about 1050° C., and a final rolling stage, in which a total compaction is not less than about 10% at a temperature of about 1050° C. to 850° C., and

after the rolling procedure is performed, cooling the rolled material from about 800° C. to 500° C. at an average cooling rate of at least about 150° C./min, without a solution treatment.

4. An austenitic stainless hot-rolled steel material having a superior corrosion resistance, a proof stress, and a low-temperature toughness, wherein a content of intermetallic compounds contained in the steel material is at most about 0.5 mass %, about 0.2% proof stress at a room temperature is at least about 550 MPa, a Charpy impact value measured using a V-notch test piece at about -40° C. is at least about 100

J/cm<sup>2</sup>, a pitting potential measured in a deaerated aqueous solution of about 10% NaCl at about 50° C. (Vc'100) is at least about 500 mV as compared to a saturated solution of Ag/AgCl, and wherein the austenitic stainless hot-rolled steel material is produced by a process comprising:

performing, at a temperature of 1200° C. to 1300° C. for at least about one hour, a homogenizing-heat treatment on a material which is at least one of a cast steel or a semi-finished product of the steel material which comprises:

C: about 0.001 to 0.03 mass %,  
Si: about 0.1 to 1.5 mass %,  
Mn: about 0.1 to 3.0 mass %,  
P: about 0.005 to 0.05 mass %,  
S: about 0.0001 to 0.003 mass %,  
Ni: about 15.0 to 21.0 mass %;  
Cr: about 22.0 to 28.0 mass %,  
Mo: about 1.5 to 3.5 mass %,  
N: about 0.15 to 0.35 mass %,  
O: about 0.0005 to 0.007 mass %, and at least one of:

W: about 0.3 to 3.0 mass %,  
Al: about 0.005 to 0.1 mass %,  
Cu: about 0.3 to 2.0 mass %,  
Sn: at most about 0.1 mass %,  
Ca: about 0.0005 to 0.0050 mass %,  
Mg: about 0.0005 to 0.0050 mass %, or  
REM: about 0.005 to 0.10 mass %,

wherein a PI value expressed by the following formula ranges from about 35 to 40: PI=Cr+3.3(Mo+0.5W)+ 30 16N,

a  $\delta$  cal value expressed by the following formula ranges from about -6 to +1:  $\delta$  cal=2.9(Cr+0.3Si+Mo+0.5W)- 35 2.6(NI+0.3Mn+0.25Cu+35C+20N)-18, and

a remnant of the steel material comprising Fe and inevitable impurities, reheating the treated material at a temperature of about 1100° C. to 1300° C.;

hot rolling the reheated material, wherein a temperature of at least about 850° C. is maintained, and the hot rolling includes a rough rolling stage, in which a total compaction is not less than about 50% at a temperature of not less than about 1050° C., and a final rolling stage, in which a total compaction is not less than about 10% at a temperature of about 1050° C. to 850° C., and

after the rolling procedure is performed, cooling the rolled material from about 800° C. to 500° C. at an average cooling rate of at least about 150° C./min, without a solution treatment.

5. An austenitic stainless hot-rolled steel material having a superior corrosion resistance, a proof stress, and a low-temperature toughness, wherein a content of intermetallic compounds contained in the steel material is at most about 0.5 mass %, about 0.2% proof stress at a room temperature is at least about 550 MPa, a Charpy impact value measured using a V-notch test piece at about -40° C. is at least about 100 J/cm<sup>2</sup>, a pitting potential measured in a deaerated aqueous solution of about 10% NaCl at about 50° C. (Vc'100) is at least about 500 mV as compared to a saturated solution of Ag/AgCl, and wherein the austenitic stainless hot-rolled steel material is produced by a process comprising:

performing, at a temperature of 1200° C. to 1300° C. for at least about one hour, a homogenizing-heat treatment on a material which is at least one of a cast steel or a semi-finished product of the steel material which comprises:

C: about 0.001 to 0.03 mass %,  
Si: about 0.1 to 1.5 mass %,

Mn: about 0.1 to 3.0 mass %,  
P: about 0.005 to 0.05 mass %,  
S: about 0.0001 to 0.003 mass %,  
Ni: about 15.0 to 21.0 mass %;  
Cr: about 22.0 to 28.0 mass %,  
Mo: about 1.5 to 3.5 mass %,  
N: about 0.15 to 0.35 mass %,  
O: about 0.0005 to 0.007 mass %, and at least one of:

10 W: about 0.3 to 3.0 mass %,

Al: about 0.005 to 0.1 mass %,

Cu: about 0.3 to 2.0 mass %,

Sn: at most about 0.1 mass %,

Ca: about 0.0005 to 0.0050 mass %,

Mg: about 0.0005 to 0.0050 mass %,

REM: about 0.005 to 0.10 mass %, or

B: about 0.0003 to 0.0060 mass %,

wherein a PI value expressed by the following formula

ranges from about 35 to 40: PI=Cr+3.3(Mo+0.5W)+

16N, and

a  $\delta$  cal value expressed by the following formula ranges from about -6 to +1:  $\delta$  cal=2.9(Cr+0.3Si+Mo+0.5W)- 2.0(NI+0.3Mn+0.25Cu+35C+20N)-18, and

25 a remnant of the steel material comprising Fe and inevitable impurities,

reheating the treated material at a temperature of about 1100° C. to 1300° C.;

hot rolling the reheated material, wherein a temperature of at least about 850° C. is maintained, and the hot rolling includes a rough rolling stage, in which a total compaction is not less than about 50% at a temperature of not less than about 1050° C., and a final rolling stage, in which a total compaction is not less than about 10% at a temperature of about 1050° C. to 850° C., and

35 after the rolling procedure is performed, cooling the rolled material from about 800° C. to 500° C. at an average cooling rate of at least about 150° C./min, without a solution treatment.

6. An austenitic stainless hot-rolled steel material having a superior corrosion resistance, a proof stress, and a low-temperature toughness, wherein a content of intermetallic compounds contained in the steel material is at most about 0.5 mass %, a Charpy impact value measured using a V-notch test piece at about -40° C. is at least about 100 J/cm<sup>2</sup>, a pitting potential measured in a deaerated aqueous solution of about 10% NaCl at about 50° C. (Vc'100) is at least about 500 mV as compared to a saturated solution of Ag/AgCl, and wherein the austenitic stainless hot-rolled steel material is produced by a process comprising:

40 performing, at a temperature of 1200° C. to 1300° C. for at least about one hour, a homogenizing-heat treatment on a material which is at least one of a cast steel or a semi-finished product of the steel material which comprises:

C: about 0.001 to 0.03 mass %,

Si: about 0.1 to 1.5 mass %,

Mn: about 0.1 to 3.0 mass %,

P: about 0.005 to 0.05 mass %,

S: about 0.0001 to 0.003 mass %,

Ni: about 15.0 to 21.0 mass %;

Cr: about 22.0 to 28.0 mass %,

Mo: about 1.5 to 3.5 mass %,

N: about 0.15 to 0.35 mass %,

O: about 0.0005 to 0.007 mass %, and at least one of:

45 W: about 0.3 to 3.0 mass %,

Al: about 0.005 to 0.1 mass %,

**39**

Cu: about 0.3 to 2.0 mass %,  
 Sn: at most about 0.1 mass %,  
 Ca: about 0.0005 to 0.0050 mass %,  
 Mg: about 0.0005 to 0.0050 mass %,  
 REM: about 0.005 to 0.10 mass %,  
 B: about 0.0003 to 0.0060 mass %,  
 Ti: about 0.003 to 0.03 mass %,  
 Nb: about 0.02 to 0.20 mass %,  
 Zr: about 0.003 to 0.03 mass %,  
 V: about 0.05 to 0.5 mass %, or  
 Ta: about 0.01 to 0.1 mass %,  
 wherein a PI value expressed by the following formula  
 ranges from about 35 to 40: PI Cr+3.3(Mo+0.5W)+16N,  
 and  
 a  $\delta$  cal value expressed by the following formula ranges 15  
 from about -6 to +1:  $\delta$  cal=2.9(Cr+0.351+Mo+0.5W)-  
 2.6(Ni+0.3Mn+0.25Cu+35C+20N)-18,

10

**40**

a remnant of the steel material comprising Fe and inevitable impurities,  
 reheating the treated material at a temperature of about  
 1100° C. to 1300° C.;  
 5 hot rolling the reheated material, wherein a temperature of  
 at least about 850° C. is maintained, and the hot rolling  
 includes a rough rolling stage, in which a total compaction  
 is not less than about 50% at a temperature of not  
 less than about 1050° C., and a final rolling stage, in  
 which a total compaction is not less than about 10% at a  
 temperature of about 1050° C. to 850° C., and  
 after the rolling procedure is performed, cooling the rolled  
 material from about 800° C. to 500° C. at an average  
 cooling rate of at least about 150° C./min, without a  
 solution treatment.

\* \* \* \* \*